# EUROPEAN PATENT APPLICATION

(11) **EP 4 782 122 A1**
(43) Date of publication of application: **29.07.2026**
(21) Application number: 24868802.0
(22) Date of filing: 19.09.2024
(51) Int. Cl.: B21D 53/88, B21D 22/02, B21D 24/00, B21D 39/02, B21D 37/16, B21D 5/02, B21D 13/02

(54) **STEEL MATERIAL FOR HOT FORMING, HOT (PRESS)-FORMED MEMBER (PART), MANUFACTURING METHOD THEREFOR, FORMING APPARATUS, FORMING METHOD, BRACKET FOR BATTERY CASE, AND BATTERY PACK MODULE**

(30) Priority: 18.09.2023 KR 20230124192; 18.09.2023 KR 20230124229; 15.12.2023 KR 20230183658; 15.12.2023 KR 20230183769; 15.12.2023 KR 20230183794; 15.12.2023 KR 20230183865
(71) Applicant: POSCO Co., Ltd, Gyeongsangbuk-do 37859 (KR)
(72) Inventor: LEE, Sea-Woong, Gwangyang-si, Jeollanam-do 57807 (KR); KIM, Hong-Gee, Incheon 21985 (KR); BOK, Hyun-Ho, Incheon 21985 (KR); OH, Kyung-Seok, Incheon 21985 (KR); LEE, Sang-Cheol, Gwangyang-si, Jeollanam-do 57807 (KR); KANG, Dae-Young, Gwangyang-si, Jeollanam-do 57807 (KR); SON, Hyun-Sung, Incheon 21985 (KR); KIM, Seong-Woo, Gwangyang-si, Jeollanam-do 57807 (KR); JUNG, Chang-Gyun, Incheon 21985 (KR); YUN, Jae-Young, Incheon 21985 (KR); KIM, Sang-Heon, Gwangyang-si, Jeollanam-do 57807 (KR); OH, Jin-Keun, Gwangyang-si, Jeollanam-do 57807 (KR)
(74) Representative: Meissner Bolte Partnerschaft mbB
(86) International application number: PCT/KR2024/096205
(87) International publication number: WO 2025/063828

(57) **Abstract**

One aspect of the present invention pertains to a steel material for hot forming used as a material for automobiles and the like, a hot formed member, a hot (press) formed part, and a method for manufacturing same.

In addition, another aspect of the present invention pertains to a forming apparatus and a forming method for forming high-strength steel, a bracket for a battery case formed thereby, and a battery pack module.

## Description

### Technical Field

An aspect of the present disclosure relates to a steel material for hot forming, used as a material for automobiles and the like, a hot formed member, a hot (press) formed part, and a method for manufacturing the same.

In addition, another aspect of the present disclosure relates to a forming apparatus and a forming method for forming high-strength steel, a bracket for a battery case formed thereby, and further, a battery pack module.

### Background Art

According to the demand for vehicle weight reduction and safety improvement, the application of high-strength steel is actively underway.

In portionicular, in order to improve fuel efficiency through vehicle weight reduction and to improve collision resistance and the like through ultra-high strengthening, members manufactured by a hot forming method are frequently being applied as a structural member (structural part) of vehicles, and also, a large amount of research thereinto is in progress.

The hot press forming method is a working method of heating a blank, forming the heated blank into a desired shape through press forming, and cooling it with a mold closed to manufacture a high-strength formed part.

In the hot press forming method as such, when the hot press forming method which is formed at a high temperature is used, even parts having a small radius of curvature may be formed without cracking due to excellent characteristics of an elongation of 50% or more at a high temperature at which forming is performed, and thus, the shape of formed parts which may not be secured with cold ultra-high strength may be secured. Besides, hot press formed parts manufactured by hot working (hot stamping) a blank may produce various shapes of parts as compared with conventional giga-grade cold formed materials, since forming is performed at a high temperature at which general formability is excellent.

As an example among the technologies related to hot forming, Patent Document 1 discloses a technology of heating an Al-Si plated steel sheet to 850°C or higher, forming the structure of a member into martensite by hot forming and quenching by press, and securing ultra-high strength of a tensile strength of 1600 MPa or more therefrom. In addition, Patent Document 1 discloses that corrosion resistance and point weldability may be secured without a treatment such as shot blast, due to an alloying layer and a diffusion layer formed by Fe diffusion from a base material into a plating layer during a heat treatment.

However, since Patent Document 1 discloses forming an Al-Si plating layer, Patent Document 1 requires a separate plating process, which is unfavorable in terms of economic feasibility and productivity.

Meanwhile, a non-plated material which is not plated may not improve surface quality due to a Fe-based oxidation layer produced during hot forming and necessarily requires a short blast process for removing the Fe-based oxidation layer, and thus, the cost of manufacturing parts is increased.

Thus, development of a technology for improving surface quality without performing a process such as the plating process and short blast is in demand.

In addition thereto, a hot formed member used for the purposes such as passenger protection should have collision resistance characteristics, and as a means for improving the collision resistance characteristics, it is considered as a very important matter to reduce the anisotropy of a material (member) after hot forming. For example, in the case of a car B-pillar, it may be difficult to protect passengers when collision performance is different depending on the direction due to the anisotropy of materials upon vehicle collision. Therefore, in order to secure the same collision performance in any collision, the anisotropy of materials needs to be reduced.

In addition, in order to improve collision performance of a hot formed member, securing excellent bendability after hot forming is considered as an important matter. For example, in the case of a car B-pillar, when bendability is poor upon vehicle collision, collision energy absorption capacity is lowered, and thus, it is difficult to secure collision stability. Thus, development of a technology which may have excellent strength, improve surface quality, and secure bendability of a hot formed member obtained by a hot forming method is required.

Meanwhile, the shape/ material/ thickness of parts for automotive structures are determined depending on the purpose required, such as functional structural parts, highrigidity structural parts, compression mode collision parts, and bending mode collision parts. In particular, a part which is connected to a plurality of peripheral parts while supporting a collision load in each direction has an ultra-high strength of a tensile strength of 1300 MPa or more for thinning and light weighting, and simultaneously, the wrinkle wave height of the flange portion joined to peripheral portions should be the same or smaller than an allowable standard of a product assembly line. For example, a center pillar part should withstand a collision transfer load so that the deformed structure upon side collision does not injure passengers, and spot welding should be sufficiently applied so that it has robust connectivity with peripheral parts such as internal reinforcement/ roof side rail/ side outer/ side sill. In addition, when the shape of the corresponding parts is complicated and a forming depth is deep, material inflow into the flange portion should be appropriately controlled in order to suppress occurrence of cracks during forming. Since the center pillar part as exemplified above also has a deep forming depth of 100 to 150 mm, a pressing pad, a gap holder, and the like are disposed in a complicated manner for controlling material inflow during forming.

FIG. 3 illustrates an example representing changes in temperature, microstructure, and tensile strength during conventional hot press forming. As shown in FIG. 3, a conventional method of imparting an ultra-high strength of a tensile strength of 1300 MPa or more to a hot press formed part forms a hard martensite structure by austenizing a material, formed at a high temperature, and cooling the material more rapidly than a critical cooling rate through heat transfer with a mold surface maintained at a low temperature. A conventional 22MnB5 material for hot pressing is generally produced, using a temperature cycle of austenizing at 850 to 1000°C, hot forming at 650 to 850°C, and cooling to a martensite transformation end temperature of 150°C or lower at a cooling rate of a critical cooling rate of 28°C/s or more. The material is characterized in that it should be an austenite single phase in which a soft phase does not occur inside the material at the end of hot forming, and an alloy component system is designed so that austenite is all transformed into martensite during later rapid cooling.

FIG. 4 illustrates an example representing the temperature, the microstructure, and the ductility by region of the parts manufactured according to the conventional hot press forming process. As shown in FIG. 4, in the conventional 22MnB5 material, when a blank holding force is used during high draw forming, some areas of the material is in contact with a mold surface which is maintained at a low temperature of 150°C or lower to cause locally rapid cooling. As a result, since the corresponding area is hardened before the periphery and the ductility is reduced, there is a concern that a boundary portion with a peripheral region may tear during forming. Therefore, in a hot draw forming process, it is difficult to use a blank holding force or drawbead effective for controlling material inflow and suppressing wrinkles, and thus, the mold structure becomes complicated and a maximum forming depth is limited. For these reasons, in automotive body parts, for example, a hot press forming process is being mainly applied to members or channels having a shallow depth or a relatively simple shape, and is selectively applied to parts where flange wrinkles are concerned/ deep parts/ large-area parts requiring control of material inflow/ parts having complicated shapes, and the like.

In order to apply a hot press forming process to parts which are difficult to form, various manufacturers utilize a complicated mold structure using various pads and shape beads in a process, or developed and use process division of previously controlling a product shape through cold press forming and then securing a material by post-heat treatment or an irregular forming process using a material insensitive to a temperature cycle. However, a forming process using a blank holding force widely used in cold press forming is not yet actively utilized, since it is difficult to manage controls for preventing cracks.

FIG. 5 illustrates an example representing changes in temperature, microstructure, and tensile strength of a 22MnB5 material and a low-temperature heating type material during hot press forming. Recently, steel manufactures are developing materials capable of hot stamping forming with different temperature cycle than before, in order to overcome the limitations of a conventional 22MnB5 material. For example, there are a "low-temperature heating type" material for hot forming for relaxing the standards of heat resistance of the material shown in FIG. 3, a "hardenability improvement type" material for hot forming for relaxing the standards of critical cooling rate for securing material quality, and the like.

FIG. 6 illustrates an example showing changes in temperature, microstructure, and tensile strength of the 22MnB5 material and the hardenability improvement type material during hot press forming. The "hardenability improvement type" material is characterized by obtaining targeted ultra-high strength even under the conditions of a slower cooling rate than 22MnB5, by suppressing occurrence of a soft phase in a continuous cooling phase transformation diagram by changing a metallurgical composition system, as shown in FIG. 6. However, when generally, a sheet material is formed into a part, a decrease in thickness occurs in a shoulder R part having a curvature by a wall surface of the part or a mold, and when a decrease degree is large, a gap occurs between a mold surface and the material, so that there is a concern that cooling becomes slower and a target material may not be secured.

Accordingly, a method capable of manufacturing automotive filler parts having a relatively deep forming depth or large panel parts requiring control of material inflow even when a hot press forming method is used, resolving forming defects such as cracks while securing ultra-high strength, and sufficiently suppressing wrinkles formed in the flange portion for assembly with peripheral parts, is being required.

Meanwhile, a battery system used in electric vehicles uses a battery case for protecting a battery cell inside, and the battery case should guarantee collision safety performance and water tightness.

The battery case for electric vehicles is usually manufactured with expensive aluminum extrusions or sheet materials, but application of steel materials which are price competitive and easy to recycle is being attempted. However, since high-strength steel has poor formability, it is difficult to form it into a desired shape.

The high-strength steel is sometimes applied only as a straight-line parts having a simple cross-section which is formed by roll forming. When the battery case is manufactured with the straight-line parts, there is an alignment problem due to spring back of thin steel plates and parts, and thus, it is difficult to perform butt welding of the corner where two straight-line parts meet.

In order to overcome the problem, a separate part (bracket) for supporting the two straight line parts by a method of wrapping the corner area may be utilized. Since the part has a longitudinal curved portion to which a required corner angle is applied and also has a flange shape connected to the upper and lower plates of the battery pack simultaneously, it is difficult to form the portion.

FIG. 10 illustrates a schematic diagram of a side frame of the battery case, and Fig. 11 illustrates a cross-sectional view taken along the line A-A' of FIG. 10. As seen in FIGS. 10 and 11, in the side frame B-1 of the battery case, a frame B-10 should have flanges formed in the upper and lower portions in order to be connected to the upper and lower plates, and this is the same as in a bracket B-20. That is, the bracket B-20 also includes a main body B-23 and flanges B-21 and B-22 which are bendingly formed from the main body B-23. The bracket B-20 is difficult to be formed, since it includes a curved portion having a radius of curvature (R1) and also has a curved surface having a radius of curvature (R2) formed in the upper and lower portions for forming flanges.

When the parts include curves or transition of dimensions, a stretch flange or shrink flange is formed on the surfaces of the flanges B-21 and B-22 depending on the morphological characteristics of the portion. In addition, two types of flanges may be simultaneously formed in the state in which one type is dominant. In the stretch flange area involving thickness reduction, when a forming amount is excessively large or formability a material is insufficient as compared with the shape required in the parts, necking which is a phenomenon of local cross-sectional area reduction due to plastic instability or a subsequent rupture problem may occur. Meanwhile, in the shrinkage flange area, a thickness increases due to an in-plane compressive load increase and buckling and wrinkle problems may occur. When the wrinkles or folding occurs, a non-uniform gap is formed in the battery pack, which may damage the water tightness of the battery pack.

Meanwhile, in order to guarantee the strength uniformity and collision safety performance in the bracket B-20, the bracket should be formed with the same material as the frame B-10 which is a straight-line part, and when it is formed with a high-strength steel, it is extremely difficult to form a flange having a curved portion.

In the case of a common steel sheet for cold forming, when it becomes an ultra-high-strength steel having a tensile strength of 980 MPa or more, there is increased risks of wrinkles and rupture due to the high strength and insufficient ductility of materials, flange working of the curved portion becomes difficult, and thus, the use of a press-hardened steel as a substitute is increasing.

Since the press-hardened steel is formed at a high temperature, it has low strength at the time of forming and rich ductility and may be formed into a complicated shape. However, since the forming should be performed at once while maintaining a high temperature, it is difficult to apply a blank holder or drawbead which is a rupture and wrinkle control means, and thus, there is a limitation in terms of a freedom degree of forming method.

Besides, though a high-strength steel generally has a problem of being incapable of forming parts having a small radius of curvature due to poor bendability, due to the recent issues of improving vehicle weight reduction and safety in electric vehicles and the like, formed parts, which has high strength but a small radius of curvature as compared with the conventional portions, and thus, are easier to use a space, are required.

Meanwhile, since in the hot press forming method, forming should be completed before a high-temperature material heated in a heating furnace is cooled in the air, forming is not performed sequentially through several stages of molds as used in cold forming. Due to the demerits, it is also difficult to form a plurality of parts having a hat shape by the hot press forming method. Since the forming is not performed at once, a method of separately forming and then attaching to each other in an assembly step may be used, but working costs may be increased due to performance and separate forming of each part.
(Patent Document 1) U.S. Patent Registration No. 6296805
(Patent Document 2) U.S. Patent Publication No. 2014-0056754
(Patent Document 3) Korean Patent Laid-Open Publication No. 10-2020-006635
(Patent Document 4) Korean Patent Laid-Open Publication No. 10-2023-0092430

### Summary of Invention

### Technical Problem

A first aspect of the present disclosure is to provide a steel material for hot forming which has excellent surface quality and may significantly lower anisotropy of materials, while a hot formed member obtained by hot forming has high strength, a hot formed member manufactured using the same, and a method for manufacturing them.

A second aspect of the present disclosure is to provide a hot formed member having excellent surface quality and improved bendability while having high strength, and a method for manufacturing the same.

A third aspect of the present disclosure is to provide a hot press formed part which may reduce wrinkles of a flange portion while securing ultra-high strength, and a method for manufacturing the same.

A fourth aspect of the present disclosure is to provide a forming apparatus capable of forming a bracket having a flange and a curved portion formed, a forming method, and a bracket manufactured thereby.

A fifth aspect of the present disclosure is to provide a formed part having a small radius of curvature while having higher tensile strength than conventional parts, or a battery pack module including the same.

A sixth aspect of the present disclosure is to provide a press formed part having significantly decreased occurrence of damages such as cracks, during hot press forming for manufacturing a plurality of parts having a hat shape, and a method for manufacturing the same.

An object of the present disclosure is not limited to the above description. Additional objects of the present disclosure are described throughout the specification, and any person with ordinary skill in the art to which the present disclosure pertains has no difficulty in understanding of the additional object of the present disclosure from the description in the specification of the present disclosure.

### Solution to Problem

Hereinafter, the technical solutions of the present disclosure will be described. Though not essential, it should be noted that the technical solution according to each aspect of the present disclosure may be useful in the technical solution of other aspects. For example, the steel material for hot forming and/or the manufacturing method thereof according to the first aspect may be useful for the hot formed member, various parts obtained therefrom, and the manufacturing method thereof according to the second to sixth aspects. Besides, the method for manufacturing parts or the heat treatment conditions used therein according to the second and third aspects may be useful in the process of manufacturing the bracket for a battery case or the formed part, and the like according to the fourth to sixth aspects. In addition, the composition and the various useful parameters according to each aspect of the present disclosure may be appropriately combined with other aspects to obtain favorable effects.

According to a first aspect of the present disclosure, a steel material for hot forming is provided, wherein a strength of a rotated-cube texture on an orientation distribution function (ODF) map is 2.50 or less, and a colony of surfaces perpendicular to the <111> direction in the thickness direction is more than 6.00% of an entire texture area.

According to an example embodiment of the present disclosure, anisotropy may be lowered, and surface quality may be excellently secured, by controlling a strength of the texture and a colony area of the surfaces perpendicular to the <111> direction in the thickness direction.

In an example embodiment of the present disclosure, the steel material for hot forming may include, by weight: 0.040 to 0.450% of carbon (C), 0.80 to 3.00% of silicon (Si), 4.00% or less (excluding 0%) of manganese (Mn), 0.050% or less of phosphorus (P), 0.0200% or less of sulfur (S), 0.010 to 0.100% of aluminum (Al), 1.000 to 5.000% of chromium (Cr), 0.020% or less (excluding 0%) of nitrogen (N), a reminder of Fe, and unavoidable impurities.

According to another example embodiment of the present disclosure, the steel material for hot forming may further include one or more elements selected from the following a) to f):
a) 0.005 to 0.400 wt% of one or more selected from titanium (Ti), niobium (Nb), zirconium (Zr), and vanadium (V),
b) 0.0001 to 0.0100 wt% of boron (B),
c) 0.001 to 1.000 wt% of one or more of molybdenum (Mo) and tungsten (W),
d) 0.003 to 2.000 wt% of one or more of copper (Cu) and nickel (Ni),
e) 0.001 to 1.000 wt% of one or more of antimony (Sb) and tin (Sn), and
f) 0.0001 to 0.0200 wt% of rare earth elements (REM).

According to another example embodiment of the present disclosure, a microstructure of the steel material for hot forming may include ferrite or a composite structure of ferrite and cementite as a main phase, and also one or more of pearlite, bainite, and martensite, and may include the main phase at an area fraction of 30% or more.

According to another aspect of the present disclosure, a method for manufacturing a steel material for hot rolling includes: preparing a steel slab; heating the steel slab in a temperature range of 1000 to 1300°C; performing finish hot rolling of the heated steel slab in a temperature range of Ar3 to 1000°C to obtain a hot rolled steel sheet; after the finish hot rolling, performing cooling at a cooling rate of 20 to 100°C/s; after the cooling, performing coiling in a temperature range of higher than Ms and 750°C or lower; after the coiling, performing cold rolling to obtain a cold rolled steel sheet; and annealing the cold rolled steel sheet in a temperature range of 700 to 900°C.

In an example embodiment of the present disclosure, the cold rolling may be performed at a rolling reduction rate of 5% or more and less than 35% in a first cold rolling mill and at a rolling reduction rate of 0.1% or more and less than 10.0% in a last cold rolling mill.

According to an example embodiment of the present disclosure, an effect of improving material anisotropy may be obtained by controlling a cold rolling process under certain conditions.

According to another aspect of the present disclosure, a hot formed member is provided, wherein the following [Equation 1] satisfies 15 or less: [Equation 1] {|Bending angle in rolling perpendicular direction - bending angle in rolling direction|/bending angle in rolling direction}×100.

In an example embodiment of the present disclosure, a microstructure of the hot formed member may be a martensite single phase or a composite structure of bainite at an area fraction of 40% or less and a remainder of martensite.

Though not essential, the steel sheet or the hot formed member according to the first aspect of the present disclosure may secure improved performance, when combined with favorable characteristics of other aspects described later.

According to a second aspect of the present disclosure, a hot formed member wherein the number of cementites having a Cr content of 1.20% or more and a length of a short diameter of 100 nm or more is 10.00/µm² or less at a point of t/4 in a thickness direction (wherein t is a thickness (mm) of the member) is provided.

According to an example embodiment of the present disclosure, bendability of the hot formed member may be improved by controlling the number of cementites having Cr at or above a certain content and a certain length or more of a short diameter.

In an example embodiment of the present disclosure, the hot formed member may be obtained from the steel material for hot forming described above.

In an example embodiment of the present disclosure, the hot formed member may include, by weight: 0.040 to 0.450% of carbon (C), 0.80 to 3.00% of silicon (Si), 4.00% or less (excluding 0%) of manganese (Mn), 0.050% or less of phosphorus (P), 0.0200% or less of sulfur (S), 0.010 to 0.100% of aluminum (Al), 1.00 to 5.00% of chromium (Cr), 0.020% or less (excluding 0%) of nitrogen (N), a reminder of Fe, and unavoidable impurities.

In an example embodiment of the present disclosure, the hot formed member may further include one or more elements selected from the following a) to f):
a) 0.005 to 0.400 wt% of one or more selected from titanium (Ti), niobium (Nb), zirconium (Zr), and vanadium (V),
b) 0.0001 to 0.0100 wt% of boron (B),
c) 0.001 to 1.000 wt% of one or more of molybdenum (Mo) and tungsten (W),
d) 0.003 to 2.000 wt% of one or more of copper (Cu) and nickel (Ni),
e) 0.001 to 1.000 wt% of one or more of antimony (Sb) and tin (Sn), and
f) 0.0001 to 0.0200 wt% of rare earth elements (REM).

In an example embodiment of the present disclosure, a microstructure of the hot formed member may be a martensite single phase or a composite structure of bainite at an area fraction of 50% or less and a remainder of martensite may be provided.

In an example embodiment of the present disclosure, a maximum bending angle of the hot formed member may be 40° or more.

In an example embodiment of the present disclosure, a standard glossiness of the hot formed member may be 25.0 GU or more.

According to another aspect of the present disclosure, a method for manufacturing a hot formed member includes: preparing a blank using a steel material; charging the blank into a furnace having a dew point of -15 to -20°C, and heating the blank at a temperature of Ae3 or higher and maintaining the temperature; and hot forming the heated and maintained blank and cooling at a cooling rate of 10 to 1000°C/s.

In an example embodiment of the present disclosure, the steel material for obtaining the hot formed member may be the steel material for hot forming described above.

According to an example embodiment of the present disclosure, an effect of improving surface quality and bendability may be obtained by controlling conditions inside the furnace during heating and maintaining of the blank.

In an example embodiment of the present disclosure, the heating and maintaining may be performed under conditions satisfying the following Relations 1 and 2: [Relation 1] 0.722260 + (0.773168×Si) + (2.073977×Mn) + (1.667101×Cr) - (0.196843×O2) - (0.031066×DP) - (0.002384×Tfurnace) - (0.001400×ttotal) ≥ 0.8 wherein Si, Mn, and Cr are contents (wt%) of an alloy composition of the member, O₂ is an oxygen concentration (%) in the furnace, DP is a dew point temperature (°C) in the furnace, T_{furnace} is a set temperature (°C) in the furnace, and tₜₒₜₐₗ is a total heating time (sec) in the furnace,
${t}_{total} \geq - 65.79 \times ln \frac{{A}_{e 3} - {T}_{furnace} + 10}{- 961.23}$
wherein tₜₒₜₐₗ is a total heating time (sec) in the furnace, Aₑ₃ is an equilibrium temperature (°C) when transformation into austenite is completed, and T_{furnace} is a set temperature (°C) in the furnace.

In an example embodiment of the present disclosure, when the blank is charged into the furnace and heated, a residence time in the furnace may be 180 seconds or more.

In an example embodiment of the present disclosure, the cooling may be performed to the temperature range of Mf or lower.

In an example embodiment of the present disclosure, the steel material may be a cold rolled steel sheet. As an example, the cold rolled steel sheet may be the steel material for hot forming described above, and the steel material may be manufactured by the manufacturing method described above.

In an example embodiment of the present disclosure, the cold rolled steel sheet may be manufactured by: preparing a steel slab; heating the steel slab in a temperature range of 1000 to 1300°C; performing finish hot rolling of the heated steel slab in a temperature range of Ar3 to 1000°C to obtain a hot rolled steel sheet; after the finish hot rolling, performing cooling at a cooling rate of 20 to 100°C/s; after the cooling, performing coiling in a temperature range of higher than Ms and 750°C or lower; after the coiling, performing cold rolling at a cumulative rolling reduction rate of 30 to 80% to obtain a cold rolled steel sheet; and annealing the cold rolled steel sheet in a temperature range of 700 to 900°C.

Though not essential, the steel sheet or the hot formed member according to the second aspect of the present disclosure may secure improved performance, when combined with favorable characteristics of other aspects described later.

According to a third aspect of the present disclosure, a hot press formed part wherein a martensite transformation critical cooling rate is 15 to 25°C/s in a temperature section of 800 to 400°C, and a wrinkle wave height of a flange portion is 1 mm or less is provided.

According to an example embodiment of the present disclosure, a hot press formed part having ultra-high strength and reduced wrinkles of the flange portion may be provided.

In an example embodiment of the present disclosure, the hot press formed part may be obtained from the steel material for hot forming described above.

According to another aspect of the present disclosure, a method for manufacturing a hot press formed part using a mold including: an upper die; a lower punch provided in a lower center of the upper die; and a lower holder provided in a lower portion of the upper die and a side portion of the lower punch includes: austenizing a steel material; providing an austenized steel material on the lower punch and the lower holder; applying a blank holding force (F) and heat through the lower holder to support the steel material between the lower holder and the upper die simultaneously with heating; and applying pressure through the lower punch to form the steel material and cooling, wherein the steel material has a martensite transformation critical cooling rate of 15 to 25°C/s in a temperature section of 800 to 400°C.

In an example embodiment of the present disclosure, the blank holding force (F) may satisfy the following Equation 2, and P may be 1 to 10 MPa:

[Equation 2] F = P × A (wherein P is a blank holding pressure, and A is a contact area between the lower holder and the steel material).

In an example embodiment of the present disclosure, the lower holder has a minimum temperature value (Tₘᵢₙ) of 300°C.

In an example embodiment of the present disclosure, the lower holder has a maximum temperature value (Tₘₐₓ) satisfying the following Equations 3 and 4:
${T}_{max} = {T}_{blank} - \left[\left({CR}_{min}⋅w⋅ρ⋅C\right)/h\right]$ $h = A ⋅ {P}^{N}$
wherein h is a heat transfer coefficient between the steel material and the lower holder, T_{blank} is a forming temperature of the steel material, Tₘₐₓ is a maximum temperature value of the lower holder, w is a thickness of the steel material, ρ is a density of the steel material, C is a specific heat of the steel material, CRₘᵢₙ is a martensite transformation critical cooling rate, a is a heat transfer pressurization coefficient of the steel material, P is a blank holding pressure, and b is a heat transfer pressurization index of the steel material.

In an example embodiment of the present disclosure, a temperature of the remaining mold excluding the lower holder may be 300°C or lower.

Though not necessarily essential, the hot press formed part according to the third aspect of the present disclosure may secure improved performance, when combined with favorable characteristics of other aspects described later.

According to a fourth aspect of the present disclosure, a forming apparatus includes: a pad; a die disposed in an outside in a first direction of the pad; and a punch which is disposed in a lower portion of the pad and includes a main body in which a punch forming portion is formed, wherein the punch forming portion includes a linear first punch forming portion, a curved second punch forming portion having a forming portion curve radius of curvature (Rp), and a linear third punch forming portion, when viewed from the first direction; the first to third punch forming portions are continuously disposed along a second direction perpendicular to the first direction on a horizontal plane; the first to third punch forming portions include first to third extended surface forming portions on a plane perpendicular to the first direction on both sides of the first direction, first to third main body forming portions on a plane in a direction towards the pad, and first to third curved surface forming portions having a bending radius of curvature (r) between the extended surface forming portion and the main body forming portion; the pad includes pressurizing surfaces corresponding to the first to third main body forming portions; the die includes a linear first die forming portion, a curved second die forming portion having a die curve radius of curvature (Rd), and a linear third die forming portion, when viewed from the first direction; the first to third die forming portion is continuously disposed along the second direction; and when upper positions of the third main body forming portion and the third die forming portion are placed on the same plane, the first main body forming portion is placed above the upper position of the first die forming portion, when viewed in the first direction.

According to an example embodiment of the present disclosure, forming of steel having insufficient formability (for example, high-strength steel) may be allowed.

In an example embodiment of the present disclosure, the punch may further include fourth and fifth punch forming portions which are symmetrical to the second and first punch forming portions around the third punch forming portion, the die may further include fourth and fifth die forming portions which are symmetrical to the second and first die forming portions around the third die forming portion, and the pressurizing surface of the pad may also include surfaces corresponding to the main body forming portions of the fourth and fifth punch forming portions.

In an example embodiment of the present disclosure, the punch may include a support portion which supports a material before forming in the outside of the first and fifth forming portions around the third punch forming portion.

In an example embodiment of the present disclosure, the forming portion curve radius of curvature (Rp) may be smaller than the die curve radius of curvature (Rd).

In an example embodiment of the present disclosure, a length in the second direction (lp) of the third main body forming portion may be longer than a length in the second direction (ld) of the third die forming portion.

In an example embodiment of the present disclosure, the center of the die curve radius of curvature (Rd) in the second direction coincides with the center of the third main body forming portion, when viewed from the first direction, and the second and fourth punch forming portions may have an angle (θ) at which extended lines of imaginary tangents intersect at both ends of 95 to 135°, when viewed from the first direction.

In an example embodiment of the present disclosure, the first to fifth die forming portions may include first to fifth die curved surface forming portions formed into a curved surface at a relatively close position to the punch in the first direction and first to fifth plane forming portions at a relatively distant position to the punch, the curved surfaces of the first to fifth die curved surface forming portions has an elevated height as they are close to the punch, and when the upper portions of the third main body forming portion and the third die forming portion are placed on the same plane, at least a portion of the second main body forming portion may be under an upper portion of the second die forming portion, when viewed from the first direction.

In an example embodiment of the present disclosure, at least one of the punch and the die may include a cooling channel inside, and the forming portion curve radius of curvature (Rp) and the bending radius of curvature (r) may satisfy: 25 mm ≤ Rp (mm) + r (mm) ≤ 30 mm.

According to another aspect of the present disclosure, a method for forming a material includes: a material settling process of settling a material which is longer than a punch having a forming portion in a first direction in the punch; a first forming process of forming the material into a shape of a main body forming portion of the punch through a pad placed on an upper portion of the punch; and a second forming process of forming the material so that the material follows a shape of the forming portion of the punch through a die placed on an outside of the pad in the first direction, wherein in the second forming process, the die performs forming in the order of an edge portion, a center portion, and a middle portion between the center and the edge portions of the material in the first direction and in a second direction perpendicular to an up-down direction.

In an example embodiment of the present disclosure, the forming portion may include a linear first forming portion, a curved second forming portion having a forming portion curve radius of curvature (Rp), a linear third forming portion, a curved fourth forming portion having the forming portion curve radius of curvature (Rp), and a linear fifth forming portion, when viewed from the first direction, the middle portion of the die may be formed into a curved surface having a die curve radius of curvature (Rd), and the die curve radius of curvature (Rd) may be larger than the forming portion curve radius of curvature (Rp).

In an example embodiment of the present disclosure, the material may be a steel sheet, the material settling process is performed in a state in which the material is heated to an AC3 temperature or higher of the material, and a cooling process of cooling the material so as to have a martensite structure by at least one of the punch and the die may be further included.

In an example embodiment of the present disclosure, the material may be the steel material for hot forming described above or a hot formed member obtained by hot forming the material for hot forming. As an example, the steel material for hot forming and the hot formed member may have the alloy composition described above and may be manufactured by the manufacturing method described above.

In an example embodiment of the present disclosure, in the material settling process, the material may include a notch formed toward the center of the material in the first direction at a position corresponding to the center portion of the die.

In an example embodiment of the present disclosure, the first to fifth forming portions may include first to fifth extended surface forming portions on a surface perpendicular to the first direction on both sides of the first direction, first to fifth main body forming portions on a surface in a direction toward the pad, and first to fifth curved surface forming portions having a bending radius of curvature (r) between the extended surface forming portion and the main body forming portion, and the forming portion curve radius of curvature (Rp) and the bending radius of curvature (r) may satisfy: 25 mm ≤ Rp (mm) + r (mm) < 30 mm, 3 mm ≤ r (mm) ≤ 10 mm.

According to another aspect of the present disclosure, a bracket for a battery case includes: a formed surface having a forming portion curve radius of curvature (Rp), wherein the formed surface includes a main body; a flange which is bendingly extended from the end of the main body; and a curved surface connecting the main body and the flange with a bending radius of curvature (r), the bracket is formed of a steel material including boron having a tensile strength of 1200 MPa or more, includes a martensite structure, and has a forming portion curve radius of curvature (Rp) and a bending radius of curvature (r) satisfying: 25 mm ≤ Rp (mm) + r (mm) ≤ 30 mm, 3 mm ≤ r (mm) ≤ 10 mm.

In an example embodiment of the present disclosure, a minimum thickness (tmin) and an initial thickness before forming (tini) in the flange may satisfy: (tini - tmin)/tini ≤ 0.2, and a maximum thickness (tmax) and an initial thickness before forming (tini) in the curved surface may satisfy (tini - tmax)/tini ≥ -0.4.

In an example embodiment of the present disclosure, the bracket may have an angle (θ) at which extended lines of imaginary tangents intersect at both ends of the formed surface of 95° to 135°.

The bracket for a battery case according to an example embodiment of the present disclosure may be manufactured by the forming method described above.

According to an example embodiment of the present disclosure, the weight reduction, water tightness, and collision safety performance of the battery pack may be secured through the bracket manufactured by the forming method described above.

Though not necessarily essential, the article according to the fourth aspect of the present disclosure may secure further improved performance by combination with favorable characteristics of other aspects described later.

According to a fifth aspect of the present disclosure, a hot press formed part of high-strength steel includes: a first wall extended in a first direction, a second wall extended in a direction intersecting the first wall, and a third wall extended in the first direction and in a direction intersecting the second wall, wherein a curvature portion is formed between the first wall and the second wall, and the first wall, the second wall, and the curvature portion are integrally formed and satisfy the following Relation 3:
[Relation 3] Height (hw) of wall portion ≤ 13.4 * angle (θw) of wall portion + 182.4 wherein the height (hw) of wall portion is a length from the first wall to the third wall in a direction perpendicular to the first direction and is in a mm unit, the angle (θw) of the wall portion is an angle between an arbitrary line perpendicular to the first direction and the second wall and is in a degree unit, and calculation is performed by making the left and right sides dimensionless.

In an example embodiment of the present disclosure, the high-strength steel may be the steel material for hot forming described above.

According to an example embodiment of the present disclosure, a formed part having a high tensile strength and a small curvature may be provided.

In an example embodiment of the present disclosure, the first wall, the second wall, and the curvature portion may be integrally formed by working a sheet material. In addition, the first wall, the second wall, and the curvature portion may be integrally formed by working the sheet material, the radius of curvature (r) of the curvature portion may be 0.55 mm or more, and a ratio (r/t) of the radius of curvature (r) to the thickness (t) of the sheet material may be less than 2.5.

In an example embodiment of the present disclosure, the formed part may have the tensile strength of 1300 to 2100 MPa.

In an example embodiment of the present disclosure, the formed part may include a third wall and a fourth wall parallel to the first direction, and a fifth wall connected to the third wall and the fourth wall, the third wall is extended from the second wall, and the first wall and the fifth wall may be integrally formed.

In an example embodiment of the present disclosure, an angle between an arbitrary line perpendicular to the first direction and the second wall may be 5° or less.

In an example embodiment of the present disclosure, a microstructure of the formed part may be formed of martensite at 98% or more of an area fraction.

According to another aspect of the present disclosure, a battery pack module includes: a battery case formed around a battery pack, a base which is placed in a lower portion of the battery case and is connected to the battery case to form a space where the battery pack is placed, and a hot press formed portion which is placed across an inside of the battery case and is connected to the battery case and the base.

According to an example embodiment of the present disclosure, a part having a high space utilization may be manufactured when manufacturing a module such as a battery pack.

In an example embodiment of the present disclosure, the hot press formed part may be disposed in multiples at regular intervals in the battery case.

Though not necessarily essential, the portion according to the fifth aspect of the present disclosure may secure further improved performance by combination with favorable characteristics of other aspects described later.

According to a sixth aspect of the present disclosure, a press formed part includes: a top plate portion, a vertical wall portion consecutive to the top plate portion, a plurality of deformation portions which has a hat shape including a boundary portion consecutive to the vertical wall portion and has a predetermined height, and flat plate portions which are disposed between the plurality of deformation portions, connect the two adjacent boundary portions, and have a predetermined length.

In an example embodiment of the present disclosure, a relationship between the predetermined length and the predetermined height may be determined based on the number of the deformation portions.

In an example embodiment of the present disclosure, three deformation portions may be provided, and a relationship between the predetermined length and the predetermined height may be defined by the following Equation (1): w≤114.85e^{0.0455h} ... Equation (1), wherein w is the predetermined length, and h is a predetermined height.

In an example embodiment of the present disclosure, four or more deformation portions may be provided, and a relationship between the predetermined length and the predetermined height may be defined by the following Equation (2): w≤46.309e^{0.105h} ... Equation (2), wherein w is the predetermined length, and h is a predetermined height.

In an example embodiment of the present disclosure, the predetermined length (w) may be 20 mm or more.

In an example embodiment of the present disclosure, the press formed part may be manufactured using a hot press forming method.

In an example embodiment of the present disclosure, the hot press forming method may be the method described above.

According to another aspect of the present disclosure, a method for manufacturing a press formed part includes: supplying a metal sheet to a working position, performing first press forming of the metal sheet using a first mold provided with a plurality of first pressurizing portions and an intermediate pressurizing portion, performing second press forming of the metal sheet using the first mold and a second mold provided with a plurality of second pressurizing portions, after performing the first press forming of the metal sheet.

In an example embodiment of the present disclosure, the metal sheet may be the steel material for hot forming described above.

In an example embodiment of the present disclosure, the press forming process may use the forming apparatus described above.

In an example embodiment of the present disclosure, in the supplying of a metal sheet to a working position, the metal sheet may be supplied between the first mold and the intermediate pressurizing portion, but a center area of the metal sheet may be disposed at a position facing the intermediate pressurizing portion.

In an example embodiment of the present disclosure, in the supplying of a metal sheet to a working position, the intermediate pressurizing portion may be placed above the second mold, at the working position.

In an example embodiment of the present disclosure, in the supplying of a metal sheet to a working position, the intermediate pressurizing portion may be disposed at a position at which a height difference between the intermediate pressurizing portion and the second mold is 65% or more of the height of the press formed part.

In an example embodiment of the present disclosure, in the first press forming of the metal sheet, the intermediate pressurizing portion may be introduced into the first pressurizing portion disposed in the middle among the plurality of first pressurizing portions and press the middle area of the metal sheet.

In an example embodiment of the present disclosure, in the second press forming of the metal sheet, the second pressurizing portion may be introduced into the first pressurizing portion disposed in the outside among the plurality of first pressurizing portions and press the outer area of the metal sheet.

In an example embodiment of the present disclosure, in the first press forming of the metal sheet and in the second press forming of the metal sheet, the metal sheet may be formed using a hot press forming method.

In an example embodiment of the present disclosure, between the first press forming of the metal sheet and the second press forming of the metal sheet, press forming the metal sheet using an additional intermediate pressurizing portion disposed in the outside of the middle pressurizing portion and the first mold may be further included.

### Advantageous Effects of Invention

According to an aspect of the present disclosure, a hot formed member having excellent surface quality and excellent anisotropy while having high strength after hot forming may be provided. Besides, a steel material for hot forming for obtaining the hot formed member and a method for manufacturing the steel material and a member may be provided.

According to another aspect of the present disclosure, a hot formed member having excellent bendability while having high strength after hot forming may be provided. Furthermore, the hot formed member according to the present disclosure may have excellent surface quality.

According to another aspect of the present disclosure, a hot press formed part which may reduce wrinkles of a flange portion while securing ultra strength and a method for manufacturing the same may be provided.

According to another aspect of the present disclosure, a forming apparatus capable of forming a bracket having a flange and a curved portion formed, a forming method, and a bracket manufactured thereby may be provided, and the weight reduction, the water tightness, and the collision safety performance of a battery pack may be secured by the bracket.

According to another aspect of the present disclosure, a formed part which has a high tensile strength and a small curvature and may be manufactured at once to be convenient for working may be provided, and also, a part having a high space utilization when manufacturing a module such as a battery pack may be manufactured.

According to another aspect of the present disclosure, intermediate pressurizing portions having a height difference are disposed between upper/lower molds, and press forming may be performed on a metal sheet using three pressurizing portions. Herein, through a stepwise forming process of first pressing the center area of the metal sheet and then sequentially pressing the outer area, concentration of strain at a specific position of the metal sheet during stamping may be prevented. Thus, the press formed part is prevented from being damaged in the manufacturing process, and part quality may be improved.

Various and beneficial merits and effects of the present disclosure are not limited to the descriptions above and may be more easily understood in a process embodiment describing specific example embodiments of the present disclosure.

### Brief Description of Drawings

FIG. 1 is a drawing showing results of ODF measurement of steel materials for hot forming of Inventive Example 1 and Comparative Example 1 according to an example embodiment of the present disclosure.
FIG. 2 is a photograph observing a surface of a hot formed member according to an example embodiment of the present disclosure.
FIG. 3 shows changes in temperature, microstructure, and tensile strength during conventional hot press forming.
FIG. 4 illustrates an example representing the temperature, the microstructure, and the ductility by region of the parts manufactured according to the conventional hot press forming process.
FIG. 5 illustrates an example representing changes in temperature, microstructure, and tensile strength of a 22MnB5 material and a low-temperature heating type material during hot press forming.
FIG. 6 illustrates an example showing changes in temperature, microstructure, and tensile strength of the 22MnB5 material and the hardenability improvement type material during hot press forming.
FIG. 7 illustrates an example showing changes in temperature, microstructure, and tensile strength of the hardenability improvement type material during hot press forming.
FIG. 8 is a schematic diagram showing hot press forming equipment which may be applied to the present disclosure.
FIG. 9 is a schematic diagram showing hot press forming equipment applied to the conventional 22MnB5 material.
FIG. 10 is a schematic diagram of a side frame of a battery case.
FIG. 11 is cross-sectional view of line A-A' of FIG. 10.
FIG. 12 is an exploded perspective view of a forming apparatus according to an example embodiment of the present disclosure.
FIG. 13 is a side view of the forming apparatus according to an example embodiment of the present disclosure.
FIG. 14 is a flowchart of a forming method according to an example embodiment of the present disclosure.
FIG. 15 is a plan view of a material added to the forming apparatus according to an example embodiment of the present disclosure.
FIG. 16 is a schematic perspective view illustrating a first forming process in the forming method according to an example embodiment of the present disclosure.
FIG. 17 is a schematic perspective view illustrating a second forming process in the forming method according to an example embodiment of the present disclosure.
FIG. 18a is a perspective view of the second forming process viewed from another direction in the forming method according to an example embodiment of the present disclosure, and FIG. 18b is a front view illustrating the second forming process in the forming method according to an example embodiment of the present disclosure.
FIG. 19 is a front view illustrating a cooling process in the forming method according to an example embodiment of the present disclosure.
FIG. 20 is a perspective view illustrating a trimming process in the forming method according to an example embodiment of the present disclosure.
FIG. 21 is a perspective view of a bracket manufactured by the forming method according to an example embodiment of the present disclosure.
FIG. 22 is a distribution chart of a thickness reduction rate of a formed article manufactured by the forming method according to an example embodiment of the present disclosure.
FIG. 23 is a distribution chart of a thickness reduction rate of a formed article manufactured by a forming method of Comparative Example 1.
FIG. 24 is a thickness reduction rate distribution graph in a cross-section of the formed articles of FIGS. 22 and 23.
FIG. 25 is a side view illustrating a forming method of Comparative Example 2.
FIG. 26 is a perspective view of a formed article manufactured by the forming method of Comparative Example 2.
FIG. 27 is a perspective view of a formed part according to an example embodiment of the present disclosure.
FIG. 28 is a front view of a formed part according to an example embodiment of the present disclosure.
FIGS. 29a, 29b, 30a, and 30b are drawings showing interpretation based on the example and the comparative example of the present disclosure, and referring to Table 1, FIG. 29a illustrates Inventive Illustration 2-1, FIG. 29b illustrates Comparative Illustration 2-1, FIG. 30a illustrates Inventive Illustration 2-3, and FIG. 30b illustrates Comparative Illustration 2-3.
FIG. 31 is a perspective view of a battery pack module according to an example embodiment of the present disclosure.
FIG. 32 which expresses a cross section of a portion of the battery pack module according to an example embodiment of the present disclosure is a drawing for showing a space utilization when the battery pack is disposed, in which (a) shows the case in which a radius of curvature is small, and (b) shows the case in which a radius of curvature is larger than that of (a).
FIG. 33 is a perspective view illustrating a press formed part according to an example embodiment of the present disclosure.
FIG. 34 is a perspective view illustrating a press formed part according to another example embodiment of the present disclosure.
In FIG. 35, (a) is a graph showing a relationship between a predetermined length and a predetermined height of the press formed part according to an example embodiment of the present disclosure, and (b) is a graph showing a relationship between a predetermined length and a predetermined height of the press formed part according to another example embodiment of the present disclosure.
In FIG, 36, (a) illustrates an example showing a strain force applied to the press formed part manufactured using a conventional manufacturing method, and (b) illustrates an example showing a strain force applied to the press formed part manufactured using the manufacturing method according to the example embodiments of the present disclosure.
FIG. 37 is a flow chart showing the method for manufacturing a press formed part according to an example embodiment of the present disclosure.
FIG. 38 schematically illustrates a first process of manufacturing the press formed part of FIG. 33.
FIG. 39 schematically illustrates a second process of manufacturing the press formed part of FIG. 33.
FIG. 40 schematically illustrates a third process of manufacturing the press formed part of FIG. 33.
FIG. 41 schematically illustrates a fourth process of manufacturing the press formed part of FIG. 33.
FIG. 42 schematically illustrates a first process of manufacturing the press formed part of FIG. 34.
FIG. 43 schematically illustrates a second process of manufacturing the press formed part of FIG. 34.
FIG. 44 schematically illustrates a third process of manufacturing the press formed part of FIG. 34.
FIG. 45 schematically illustrates a fourth process of manufacturing the press formed part of FIG. 34.

### Best Mode for Invention

As described above, the hot formed member used as a material for automobiles and the like needs to improve collision resistance, and the present inventors recognized that securing anisotropy of a material or securing bendability of a material are important matters in improving the collision resistance of the hot formed member.

Thus, the present inventors conducted in-depth research, and as a result, confirmed that a hot formed member obtained by hot forming has high strength and low anisotropy to be favorable for collision resistance, and furthermore, a steel material for hot forming having improved surface quality and a hot formed member obtained using the same may be provided, thereby completing the present disclosure.

Besides, the present inventors confirmed that a hot formed member having excellent bendability may be provided, thereby providing the present disclosure.

Hereinafter, the present disclosure will be described in detail.

The steel material for hot forming according to the first aspect of the present disclosure may include, by weight: 0.040 to 0.450% of carbon (C), 0.80 to 3.00% of silicon (Si), 4.00% or less (excluding 0%) of manganese (Mn), 0.050% or less of phosphorus (P), 0.0200% or less of sulfur (S), 0.010 to 0.100% of aluminum (Al), 1.00 to 5.00% of chromium (Cr), and 0.020% or less (excluding 0%) of nitrogen (N).

Hereinafter, the reasons for limiting an alloy composition of the steel material and the member according to an example embodiment of the present disclosure will be described in detail. Meanwhile, unless otherwise particularly stated, the content of each element is by weight and the ratio of the structure is by area.

### Carbon (C): 0.040 to 0.450%

Carbon (C) is an essential element which is added for improving strength of a hot formed member obtained by hot formed member. When the content of C is less than 0.040%, it is difficult to secure sufficient strength, and collision energy absorption capacity is reduced. Meanwhile, when the content of C is more than 0.450%, it is favorable for securing the strength of the hot formed member, but bendability is reduced to lower the collision energy absorption capacity.

Therefore, according to an example embodiment of the present disclosure, C may be included at 0.0040 to 0.450%, according to another example embodiment, at 0.050% or more, and according to still another example embodiment, at 0.400% or less.

### Silicon (Si): 0.80 to 3.00%

Silicon (Si) is concentrated on the surface when the obtained cold rolled sheet is annealed in a continuous annealing line and plays an important role in forming a Si-based amorphous oxide layer, and also, suppresses formation of a (Fe, Mn, Cr)-based oxide layer in a hot forming process and plays an important role in securing point weldability of the hot formed member.

When the content of Si is less than 0.80%, the effects described above may not be sufficiently obtained, but when the content is more than 3.00%, a Si-based amorphous oxide layer is formed to be too thick to rather reduce the point weldability.

Therefore, according to an example embodiment of the present disclosure, Si may be included at 0.80 to 3.00%, and according to another example embodiment, at 0.85% or more and 2.80% or less. According to another example embodiment, Si may be included at 2.50% or less.

### Manganese (Mn): 4.00% or less (excluding 0%)

Manganese (Mn) may secure a solid solution strengthening effect of a steel, and also, is effective for suppressing formation of ferrite during hot forming through hardenability improvement. When the content of Mn is more than 4.0%, the strength of a steel material is increased to reduce cold rollability, and a band-like structure arranged in a rolling direction on a microstructure deepens to deteriorate a collision energy absorption capacity.

According to an example embodiment of the present disclosure, the lower limit of the Mn content is not particularly defined, and when added at more than 0%, the present disclosure may be reached.

According to another example embodiment of the present disclosure, Mn may be included at 0.10% or more, and according to another example embodiment, at 0.30% or more.

### Phosphorus (P): 0.05% or less

Phosphorus (P) is an impurity which is unavoidably added in a steel manufacturing process, and when the content is more than 0.05%, the weldability of the hot formed member may be greatly impaired. Since P is an avoidable impurity, the lower limit of the content is not particularly defined. However, since high manufacturing costs may be required for controlling the content of P to less than 0.001%, the content may be 0.001% or more considering this.

### Sulfur (S): 0.0200% or less

Sulfur (S) is an impurity which is unavoidably added in a steel manufacturing process, and an element which impairs the ductility, impact characteristics, and weldability of the hot formed member. Thus, it is favorable that the content is limited to a maximum of 0.0200%. Since S is an avoidable impurity, the lower limit of the content is not particularly defined. However, since high manufacturing costs may be required for controlling the content of S to less than 0.0001%, the content may be 0.0001% or more considering this.

### Aluminum (Al): 0.010 to 0.100%

Aluminum (Al) is an element which deoxidizes in a steel making process to increase cleanliness of a steel. In order to sufficiently obtain the effect described above, it is favorable that Al is included at 0.010% or more, and when the content is more than 0.100%, high-temperature ductility is reduced by AlN which is excessively formed during continuous casting, resulting in occurrence of slab cracks.

According to an example embodiment of the present disclosure, Al may be included at 0.010 to 0.100%.

### Chromium (Cr): 1.000 to 5.000%

Chromium (Cr) is favorable for securing hardenability of a steel, like Mn, and in the present disclosure, is added for securing a good-looking surface during a hot forming process. When the content of Cr is less than 1.000%, it is difficult to secure a good-looking surface after hot forming, but when the content is more than 5.000%, a hardenability improvement effect as compared with the added amount is insignificant, and formation of a coarse Cr-based carbide is encouraged to deteriorate the collision energy absorption capability of the member.

According to an example embodiment of the present disclosure, Cr may be included at 1.000 to 5.000%. According to another example embodiment of the present disclosure, Cr may be included at 1.100% or more, and according to another example embodiment, at 4.800% or less.

### Nitrogen (N): 0.020% or less (excluding 0%)

Nitrogen (N) is an element which is unavoidably added to a steel, and when the content of N is more than 0.020%, N is bonded to Al in the steel to form AlN, which facilitates slab crack occurrence. Since N is an avoidable impurity, the lower limit of the content is not particularly defined. However, since high manufacturing costs may be required for controlling the content of N to less than 0.001%, the content may be 0.001% or more considering this.

In an example embodiment of the present disclosure, a remaining component other than the components described above is iron (Fe). However, since in a common manufacturing process, unintended impurities may be unavoidably incorporated from raw materials or the surrounding environment, the component may not be excluded. Since these impurities are known to any person skilled in the common manufacturing process, the entire contents thereof are not particularly mentioned in the present specification.

The steel material for hot forming and the member according to an example embodiment of the present disclosure may further include one or more selected from the following elements, that is, the following a) to f). By optionally adding the element, characteristics such as hot formability together with the surface quality of the steel may be further improved.

### a) 0.005 to 0.400 wt% of one or more selected from titanium (Ti), niobium (Nb), zirconium (Zr), and vanadium (V)

Titanium (Ti), niobium (Nb), zirconium (Zr), and vanadium (V) improve strength of the hot formed member by forming microprecipitates in steel, and simultaneously are effective for improving stabilization and impact toughness of retained austenite by crystal grain refinement.

In including one or more of the elements, when the content is less than 0.005%, the effect described above may not be sufficiently obtained, but when the content is more than 0.400%, the intended effect may be saturated, and also excessive addition of alloy elements leads to an increase in costs.

In an example embodiment of the present disclosure, when one or more of the elements are included, they may be included at 0.005 to 0.400%. In another example embodiment of the present disclosure, the content may be 0.008% or more in terms of the lower limit of the content of the elements and may be 0.380% or less or 0.350% or less in terms of the upper limit of the content.

In another example embodiment of the present disclosure, when only one of the elements is included, 0.005 to 0.100% of Ti, 0.005 to 0.100% of Nb, 0.005 to 0.100% of Zr, or 0.005 to 0.100% of V may be included.

### b) Boron (B): 0.0001 to 0.0100%

Boron (B) may improve the hardenability of steel only with a small amount of addition and also is segregated in an prior austenite crystal grain boundary, and thus, is useful for suppressing brittleness of a hot formed member by grain boundary segregation of P and/or S. In the case of adding B, when the content is less than 0.0001%, the effects described above may not be sufficiently obtained, but when the content is more than 0.0100%, the effect described above is saturated, and also in the case of hot rolling, hot embrittlement may be caused.

In an example embodiment of the present disclosure, when B is added, it may be included at 0.0001 to 0.0100%. In another example embodiment of the present disclosure, B may be included at 0.00012% or more or 0.00015% or more in terms of the lower limit of the content and 0.0050% or less in terms of the upper limit of the content.

### c) 0.001 to 1.000 wt% of one or more of molybdenum (Mo) and tungsten (W)

Molybdenum (Mo) and tungsten (W) may be added for promoting strength improvement and crystal grain refinement by effects of precipitation strengthening of steel and hardenability improvement of steel. In including one or more of Mo and W, when the content is less than 0.001%, the effects described above may not be sufficiently obtained, but when the content is more than 1.000%, the effect may be saturated, and the cost may be greatly increased.

In an example embodiment of the present disclosure, when one or more of the elements are included, they may be included at 0.001 to 1.000%. In another example embodiment of the present disclosure, when one or more of the elements are included, the content may be 0.0015% or more or 0.0020% or more in terms of the lower limit of the content, and may be 0.950% or less or 0.900% or less in terms of the upper limit of the content.

According to another example embodiment of the present disclosure, when only one of the elements is added, each may be included at 0.001 to 0.500%.

### d) 0.003 to 2.000 wt% of one or more of copper (Cu) and nickel (Ni)

Copper (Cu) serves to improve strength by forming fine precipitates in steel, and when Cu is added alone, it may cause hot embrittlement, and thus, in order to prevent this, nickel (Ni) may be added, if necessary. In including one or more of Cu and Ni, when the sum of the contents is less than 0.003%, the effects described above may not be sufficiently obtained, but when the content is more than 2.000%, an excessive increase in cost may be caused.

According to an example embodiment of the present disclosure, when one or more of the elements are included, they may be included at 0.003 to 2.000%. According to another example embodiment of the present disclosure, when one or more of the elements are included, the content may be 0.005% or more, 0.006% or more, or 0.007% or more in terms of the lower limit of the content and may be 1.950% or less or 1.900% or less in terms of the upper limit of the content.

According to another example embodiment of the present disclosure, when only one of the elements is added, each may be included at 0.003 to 1.500%.

### e) 0.001 to 1.000 wt% of one or more of antimony (Sb) and tin (Sn)

Antimony (Sb) and tin (Sn) have an effect of suppressing production of an oxide in a crystal grain boundary on the surface layer of a hot rolled material in a steel to which silicon (Si) is added, and also, when annealing a cold rolled material, dent defects due to falling off of a surface layer crystal grain boundary when annealing a cold rolled material may be suppressed. In order to obtain the effect described above, when one or more of Sb and Sn are added, they may be included at 0.001% or more. However, when the content is more than 1.000%, the costs may be greatly increased, and also the elements are solid solubilized in a slab grain boundary and are highly likely to cause edge cracks in a coil during hot rolling.

According to an example embodiment of the present disclosure, in further including the elements, they may be included at 0.001 to 1.000%, based on the sum of the contents. According to another example embodiment of the present disclosure, the content may be 0.002% or more or 0.030% or more in terms of the lower limit of the content and may be 0.950% or less or 0.900% or less in terms of the upper limit of the content.

According to another example embodiment of the present disclosure, when only one of the elements is added, each may be included at 0.001 to 0.500%.

### f) 0.0001 to 0.0200 wt% of rare earth elements (REM)

Rare earth elements (REM) may control activity of Fe in steel to control a formed thickness of Fe scale on the surface layer during hot forming. In order to obtain the effect, REM may be included at 0.0001% or more. However, when the content is more than 0.0200%, controllability of the Fe activity is lost, so that the surface quality of the hot formed member may be deteriorated.

According to another example embodiment of the present disclosure, in further including the REM, REM may be included at 0.0001 to 0.0200%. In another example embodiment of the present disclosure, the content may be included at 0.00015% or more or 0.0002% or more in terms of the lower limit of the content and 0.0100% or less in terms of the upper limit of the content.

In an example embodiment of the present disclosure, in the steel material for hot forming, a strength of a rotated-cube texture on an orientation distribution function (ODF) map may be 2.50 or less, and a colony of surfaces perpendicular to the <111> direction in the thickness direction may be more than 6.00% of an entire texture area. Herein, ODF refers to the ODF results on ferrite.

The strength of the rotated-cube texture on the ODF map and the colony area of surfaces perpendicular to the <111> direction in the thickness direction of the steel material are used as an indicator showing anisotropy.

Specifically, when the strength of the rotated-cube texture on the ODF map is more than 2.50, and the colony of the surfaces perpendicular to the <111> direction in the thickness direction is 6.00% or less of the entire texture area, the bending anisotropy after hot forming of the steel material is increased, so that the bending angle deviation in the rolling direction and the direction perpendicular to the rolling direction is more than 15.0 to deteriorate anisotropy. That is, the bending anisotropy in each direction is increased, so that collision resistance characteristics in various collision modes upon collision of the hot formed member may not be secured.

In an example embodiment of the present disclosure, a deviation in a bending angle may be measured by a 3-point bending test depending on the VDA (VDA238-100), and the results of the deviation in a bending angle may be calculated by the following [Equation 1]. When the line (surface) bent during the 3-point bending test is parallel to the rolling direction, it is represented as a bending angle of a rolling perpendicular direction (C direction), and when the bent line (surface) is perpendicular to the rolling direction, it is defined as a bending angle of the rolling direction (L direction): [Equation 1] {|Bending angle in rolling perpendicular direction - bending angle in rolling direction|/bending angle in rolling direction}×100.

In an example embodiment of the present disclosure, the microstructure of the steel material for hot forming is not particularly defined, and appropriate phases and the fraction of each phase will be determined by the alloy composition described above and the manufacturing process described later.

As an example, the microstructure of the steel material for hot forming may include ferrite or a composite structure of ferrite and cementite as a main phase. Additionally, one or more of pearlite, bainite, and martensite may be further included.

In an example embodiment of the present disclosure, when the C content is relatively low within the content range of carbon (C) contained in the steel material for hot forming, the main phase may be composed of ferrite and cementite, and the main phase may be included at an area fraction of 30% or more. Herein, when the microstructure is the composite structure of ferrite and cementite as a main phase, it refers to the sum of the fractions of the two phases.

In an example embodiment of the present disclosure, the steel material for hot forming may include one or more of pearlite, bainite, and martensite as a structure other than the main phase, and herein, the fraction of each phase is not particularly defined. However, though not necessarily limited thereto, the pearlite may be included at 30% or less, the bainite may be included at 20% or less, and the martensite may be included at 20% or less as the area fraction.

In an example embodiment of the present disclosure, the steel material for hot forming has high strength, and specifically, may have a tensile strength of 550 MPa or more.

Hereinafter, the method for manufacturing a steel material for hot forming according to another aspect of the present disclosure will be described in detail.

According to an example embodiment of the present disclosure, the steel material may be obtained by the processes such as [steel slab heating - hot rolling - cooling - coiling - cold rolling - annealing], and the steel material may be a cold rolled steel sheet obtained by a series of processes. Each process step will be described in detail, and the following manufacturing process corresponds to an example for manufacturing the steel material of the present disclosure.

### [Steel slab heating]

First, a steel slab having the alloy composition described above may be prepared and then heated, and the heating process of the steel slab is for performing a subsequent hot rolling process well. Herein, since the alloy composition of the steel slab may refer to the alloy composition of the steel material for hot forming mentioned above, the description of each element will be replaced by the above description.

In an example embodiment of the present disclosure, the heating process may be performed in a temperature range of 1000 to 1300°C. When the heating temperature of the steel slab is lower than 1000°C, it is difficult to homogenize a slab structure, but when the temperature is higher than 1300°C, an oxide is excessively formed, which is likely to cause surface defects after hot rolling. In addition, the manufacturing cost is increased.

### [Hot rolling]

The heated steel slab may be hot rolled to obtain a hot rolled steel sheet.

In an example embodiment of the present disclosure, the finish hot rolling may be performed in a temperature range of Ar3 to 1000°C. When the temperature of the finish hot rolling is lower than Ar3, a mixed structure may occur on the surface layer of the hot rolled steel sheet by two phase region rolling, and also there is a difficulty in controlling the shape of the hot rolled steel sheet. However, when the temperature is higher than 1000°C in the finish hot rolling, the crystal grains of the hot rolled steel sheet is coarsened, so that it is difficult to obtain the intended physical properties.

### [Cooling]

The hot rolled steel sheet may be cooled.

In an example embodiment of the present disclosure, the cooling may be performed at a rate of 20 to 100°C/s. When the cooling rate is less than 20°C/s during cooling after the hot rolling, formation of pearlite and cementite on the surface layer of the steel sheet is insignificant, so that strength may not be sufficiently secured after the subsequent hot forming. However, when the cooling rate is more than 100°C/s, pearlite and cementite are formed at an excessive area ratio on the surface in the subsequent annealing process, so that a hardness deviation between the surface layer martensites formed by the hot forming is increased, thereby deteriorating bendability.

In an example embodiment of the present disclosure, the cooling may be performed to the temperature of a follow-up coiling process.

### [Coiling]

The cooled hot rolled steel sheet may be coiled.

In an example embodiment of the present disclosure, the coiling may be performed in a temperature range of higher than Ms and 750°C or lower. During the coiling, when the coiling temperature is Ms or lower, the strength of the hot rolled steel sheet is raised too high, so that cold rollability is reduced. However, when the coiling temperature is higher than 750°C, an oxide layer is formed to be thick, and grain boundary oxidation is caused on the surface layer to deteriorate pickling ability, and also defects such as falling out of the surface layer grain boundary during annealing in a continuous annealing furnace may occur. Herein, Ms refers to a martensite transformation start temperature.

### [Cold rolling]

The inventors of the present disclosure recognized that when the hot forming process is performed after manufacturing a cold rolled steel sheet by the common cold rolling conditions, the anisotropy of the hot formed member is increased to increase a deviation in bendability in each direction.

Thus, the inventors intended to secure the bending anisotropy of the hot formed member obtained through a subsequent hot forming process, by optimizing the conditions of the cold rolling process.

According to an example embodiment of the present disclosure, in performing cold rolling while uncoiling the coiled hot rolled steel sheet, there is a technical significance in the cold rolling in the first cold rolling mill is controlled to a rolling reduction rate of 5% or more and less than 35%, and the cold rolling in the last cold rolling mill is controlled to a rolling reduction rate of 0.1% or more and less than 10.0%.

In an example embodiment of the present disclosure, the number of the rolling mills during the cold rolling (that is, the number of cold mill rolls) is not limited, but the cold rolling may be performed in at least 4 or more cold rolling mills, and the rolling reduction rate of the first cold rolling and the rolling reduction rate of the final cold rolling may be controlled as described above therein.

When the rolling reduction rate of the first cold rolling and the rolling reduction rate of the final cold rolling do not satisfy the set lower limit, a sufficient recrystallization driving force is not secured, and it becomes difficult to secure material anisotropy in the hot formed member. However, when each rolling reduction rate is more than the set upper limit, a recrystallization driving force may be sufficiently secured in the subsequent annealing process, and it is favorable for improving the material anisotropy, but an excessive rolling load occurs to deteriorate productivity.

That is, the rolling reduction rate of the specific cold rolling mill is controlled in the cold rolling process according to an example embodiment of the present disclosure, thereby securing an appropriate crystal orientation after the subsequent annealing, and thus, an effect of decreasing a deviation in the maximum bending angle in each direction of the hot formed member obtained after the hot forming, that is to say, an effect of securing anisotropy excellently is exhibited.

In an example embodiment of the present disclosure, when the cold rolling is performed under the conditions described above, the total reduction rate of the cold rolling is not particularly limited. As a non-limiting example, the cold rolling may be performed at the total reduction rate of 30 to 80%, and a predetermined target thickness may be secured therefrom.

In an example embodiment of the present disclosure, before the cold rolling of the coiled hot rolled steel sheet, a pickling process may be further performed, and surface quality may be further improved therefrom. Since the pickling process may be performed under common conditions, the conditions are not particularly limited.

### [Annealing]

The cold rolled steel sheet obtained by the cold rolling may be annealed.

In an example embodiment of the present disclosure, the annealing may be performed in a temperature range of 700 to 900°C. When the temperature during the annealing is lower than 700°C, it is difficult to recover and recrystallize a rolled structure produced in the cold rolling process, but when the temperature is higher than 900°C, annealing equipment may be deteriorated, which may be a factor in increasing manufacturing costs due to frequent replacement of the equipment and the like.

In an example embodiment of the present disclosure, the annealing may be performed for 1 to 1000 seconds. When the annealing time is less than 1 second, the effect of the annealing may not be obtained, but when the time is more than 1000 seconds, productivity may be reduced.

Hereinafter, the hot formed member according to another aspect will be described in detail.

The hot formed member according to an example embodiment of the present disclosure may be obtained by hot press forming the steel material for hot forming.

In an example embodiment of the present disclosure, the alloy composition of the hot formed member may be the same as the steel material for hot forming, and as an example, since the steel material for hot forming may have the alloy composition described above, the description of each element will be replaced with the above description.

In an example embodiment of the present disclosure, in the hot formed member, the following [Equation 1] may satisfy 15.0 or less: [Equation 1] {|Bending angle in rolling perpendicular direction - bending angle in rolling direction|/bending angle in rolling direction}×100.

In an example embodiment of the present disclosure, [Equation 1] is an equation defining a deviation in a bending angle of the hot formed member, and the value of [Equation 1] being more than 15.0 means that anisotropy is poor, and finally bendability or collision characteristics may be poor.

As a non-limiting example, the deviation in a bending angle may be confirmed from the 3-point bending test according to the VAD standard (VDA238-100).

In an example embodiment of the present disclosure, the hot formed member may have a martensite single phase or a composite structure of a bainite at an area fraction of 40% or less and a remainder of martensite, as a microstructure.

The martensite is a structure effective for securing targeted strength. Meanwhile, since the bainite is a structure having a somewhat lower strength than martensite, when it is formed at a specific fraction or more, the bendability of a material may be deteriorated, and also anisotropy may be adversely affected. Thus, the hot formed member according to an example embodiment of the present disclosure may include a bainite phase as a microstructure, but the fraction thereof may be 40% or less at this time. When the fraction of bainite is more than 40%, bendability and anisotropy may be deteriorated.

The hot formed member according to an example embodiment of the present disclosure may have a tensile strength of 1000 MPa or more.

Hereinafter, the method for manufacturing a hot formed member according to another aspect of the present disclosure will be described. The manufacturing method described later is only one example embodiment among all possible example embodiments, and it does not mean that the hot formed member of the present disclosure is necessarily manufactured by the following manufacturing method.

In an example embodiment of the present disclosure, a steel material for hot forming may be prepared, and a blank may be manufactured using the steel material. Herein, the steel material for hot forming may be a steel material according to an example embodiment of the present disclosure.

In an example embodiment of the present disclosure, the blank may be heated to a temperature of 700°C or higher, and the heating may be performed at a heating rate of 1 to 1000°C/s. When the heating temperature of the blank is lower than 700°C, recrystallization of ferrite may not be sufficient, so that bending anisotropy after hot forming may be increased. Meanwhile, when the heating rate is less than 1°C/s during heating to the temperature, productivity may be reduced, but when the heating rate is more than 1000°C/s, equipment requiring excessive costs may be needed.

In an example embodiment of the present disclosure, the heated blank may be hot formed into an intended shape using a mold and the like, and then the hot formed blank may be cooled. As an example, when the hot formed blank is cooled, the cooling may be performed at a cooling rate of 5 to 1000°C/s. When the cooling rate is less than 5°C/s during the cooling, unintended ferrite, a pearlite texture is formed, so that it becomes difficult to secure strength. However, when the cooling rate is more than 1000°C/s, expensive special cooling equipment is required. Herein, a cooling end temperature may be Mf or lower, and when the cooling is finished at a temperature higher than Mf, the cooling may be performed again to room temperature, and in this case, it is difficult to secure the shape fixability of the hot formed member. Herein, Mf refers to a martensite transformation end temperature.

The cooling process may be, as an example, a mold cooling method.

Meanwhile, according to a second aspect of the present disclosure, a hot formed member wherein the number of cementites having a Cr content of 1.20% or more and a length of a short diameter of 100 nm or more is 10.00/µm² or less at a point of t/4 in a thickness direction (wherein t is a thickness of the member) may be provided.

When Cr present in steel is concentrated in cementite, a remelting phenomenon may be slowed down to deteriorate the hardenability of a material. Thus, there is a technical significance in favorably securing bendability by controlling the number of cementites in which Cr is concentrated at a specific content or more.

In an example embodiment of the present disclosure, when the number of cementites having a Cr content at a point of t/4 in the thickness of the hot formed member of 1.20% or more and a length of a short diameter of 100 nm or more is more than 10.00/µm², the hardenability of the member is deteriorated, so that ferrite may be formed in a cooling process after hot forming, and a phenomenon of stress concentration into cementite becomes more severe during bending to deteriorate bendability.

The hot formed member according to an example embodiment of the present disclosure may include a martensite single phase or a composite structure of martensite and bainite, as a microstructure.

In an example embodiment of the present disclosure, when the microstructure of the hot formed member is the composite structure, the martensite phase may be included at an area fraction of 50% or more. The martensite is a structure effective for securing strength. Meanwhile, since the bainite is a structure having a somewhat lower strength than martensite, when it is formed at a specific fraction or more, bendability of the material may be deteriorated.

Thus, the hot formed member according to an example embodiment of the present disclosure may include a bainite phase as a microstructure, but the fraction thereof may be 50% or less at this time. When the fraction of bainite is more than 50%, bendability may be deteriorated.

The hot formed member according to an example embodiment of the present disclosure may have a tensile strength of 1000 MPa or more and may have characteristics of excellent bendability and surface quality.

In an example embodiment of the present disclosure, the hot formed member may have a maximum bending angle of 40° or more and a surface glossiness of 20.0 GU or more. When the surface glossiness of the hot formed member is less than 25.0 GU, surface quality is not secured, and a Fe oxide on the surface layer may be removed, and for this, a shot blasting process is essentially required.

In an example embodiment of the present disclosure, since the alloy composition of the hot formed member may have the alloy composition described above, the description of each element will be replaced with the above description.

Hereinafter, the method for manufacturing a hot formed member according to another aspect of the present disclosure, specifically, a method for manufacturing a hot formed member having excellent bendability will be described.

In an example embodiment of the present disclosure, a steel material may be prepared, and then a blank may be manufactured using the steel material. Herein, the steel material may be the steel material (steel material for hot forming) according to an example embodiment, and as a non-limiting example, since the steel material may have the alloy composition described above, the description for each element will be replaced by the above description.

In an example embodiment of the present disclosure, the blank may be charged into a furnace having a dew point of -15 to 20°C to heat the blank to a temperature of Ae3 or higher and then maintained.

According to an example embodiment, when the blank is heated and maintained, it may be performed under the conditions satisfying both the following Relations 1 and 2. That is, the blank may be stayed for the time defined by the following Relation 2, in the furnace satisfying the heat treatment conditions of the following Relation 1: [Relation 1] 0.722260 + (0.773168×Si) + (2.073977×Mn) + (1.667101×Cr) - (0.196843×O2) - (0.031066×DP) - (0.002384×Tfurnace) - (0.001400×ttotal) ≥ 0.8 wherein Si, Mn, and Cr are contents (wt%) of an alloy composition of the member, O₂ is an oxygen concentration (%) in the furnace, DP is a dew point temperature (°C) in the furnace, T_{furnace} is a set temperature (°C) in the furnace, and tₜₒₜₐₗ is a total heating time (sec) in the furnace,
${t}_{total} \geq - 65.79 \times ln \frac{{A}_{e 3} - {T}_{furnace} + 10}{- 961.23}$
wherein tₜₒₜₐₗ is a total heating time (sec) in the furnace, Aₑ₃ is an equilibrium temperature (°C) when transformation into austenite is completed, and T_{furnace} is a set temperature (°C) in the furnace.

In an example embodiment of the present disclosure, when the equipment for heating the blank is heating equipment composed of connected furnaces such as a roller hearth type furnace, T_{furnace} of Relation 2 shows the temperature of a furnace having the highest set temperature among the connected furnaces.

In an example embodiment of the present disclosure, when heating is performed for less time than the total heating time obtained from Relation 2, that is, the residence time in the furnace is less than the value of Relation 2, sufficient reverse transformed austenite may not be secured, and thus, the intended physical properties of the hot formed member may not be secured after completing the subsequent cooling process.

In an example embodiment of the present disclosure, in heating and maintaining the blank under the conditions satisfying both Relations 1 and 2, when the residence time in the furnace is less than a total of 180 seconds, reverse transformation into austenite is not sufficiently performed, so that ferrite may be included as a microstructure after the subsequent cooling process. In addition, since remelting of cementite is not actively performed, and the number of cementites having a specific amount or more of Cr and a short diameter of 100 nm or more becomes excessive to deteriorate hardenability, and thus, ferrite may exist after the cooling to deteriorate bendability. Therefore, in an example embodiment of the present disclosure, during the blank heating, the residence time in the furnace may be 180 seconds or more, according to another example embodiment, it may be set to 200 seconds or more, and according to still another example embodiment, it may be 240 seconds or more.

In an example embodiment of the present disclosure, when the dew point in the furnace is lower than -15°C, air of which the dew point is controlled should be excessively added, which may cause a rise in process costs. However, when the temperature is higher than 20°C, it becomes difficult to secure good surface quality, and an amount of diffusible hydrogen introduced during the hot forming may be increased to deteriorate bendability.

In an example embodiment of the present disclosure, an oxygen concentration (O₂) in the furnace may be 15% or less. As another example, the oxygen concentration may be 10% or less.

According to an example embodiment of the present disclosure, the heated and maintained blank may be hot formed into an intended shape using a mold and the like. Thereafter, the heat formed blank may be cooled, which may be performed at a cooling rate of 10 to 1000°C/s.

In an example embodiment of the present disclosure, when the cooling rate is less than 10°C/s during the cooling, unintended ferrite, a pearlite texture is formed, so that it becomes difficult to secure strength. However, when the cooling rate is more than 1000°C/s, expensive special cooling equipment is required.

In an example embodiment of the present disclosure, the cooling end temperature in the cooling may be Mf or lower, and when the cooling is finished at a temperature higher than Mf, the cooling may be performed again to room temperature, and in this case, it is difficult to secure the shape fixability of the hot formed member. Herein, Mf refers to a martensite transformation end temperature.

In another example of the present disclosure, in order to secure better elongation and impact resistance in the hot formed member, martensite may be tempered, and retained austenite may be stabilized by the process of stopping cooling in a temperature range of Mf to Ms and then maintaining the temperature, or a process of stopping cooling in a temperature range of Mf to Ms and then heating to Ac1 or lower again (reheating). Herein, Ms refers to a martensite transformation starting temperature, and Ac1 refers to a temperature at which transformation of ferrite + cementite into austenite starts during heating.

When the hot formed member according to an example embodiment of the present disclosure is manufactured, the steel material used for obtaining the blank may be a cold rolled steel sheet. Herein, the cold rolled steel sheet may be manufactured by the method suggested for manufacturing the steel material described above, that is, a steel material for hot forming, but is not limited thereto.

As an example, the cold rolled steel sheet may be manufactured by: preparing a steel slab; heating the steel slab in a temperature range of 1000 to 1300°C; performing finish hot rolling of the heated steel slab in a temperature range of Ar3 to 1000°C to obtain a hot rolled steel sheet; after the finish hot rolling, performing cooling at a cooling rate of 20 to 100°C/s; after the cooling, performing coling in a temperature range of higher than Ms and 750°C or lower; after the coiling, performing cold rolling at a cumulative rolling reduction rate of 30 to 80% to obtain a cold rolled steel sheet; and annealing the cold rolled steel sheet in a temperature range of 700 to 900°C. Herein, the cold rolling after the coiling may be performed at a cumulative rolling reduction rate of 30 to 80% in terms of securing a predetermined target thickness.

Hereinafter, the hot press formed part according to the third aspect of the present disclosure will be described.

FIG. 7 illustrates an example showing changes in temperature, microstructure, and tensile strength of the hardenability improvement type material during hot press forming. The hot press formed part according to an example embodiment of the present disclosure is characterized by using a hardenability improvement type material having changes in temperature, microstructure, and tensile strength during hot press forming as shown in FIG. 7, as an example. The hardenability improvement type material is characterized by obtaining ultra-high strength of 1300 MPa or more, more advantageously 1500 MPa or more even under the slower cooling rate condition than 22MnB5 which is conventionally mainly used. In addition, when a sheet material is formed into a part, a targeted material may be secured even in a thickness decrease region in a shoulder R portion having a curvature for a generally occurring product wall surface or mold.

Meanwhile, the hardenability improvement type material may have a martensite transformation critical cooling rate (CRₘᵢₙ) in a temperature section of 800 to 400°C of 15 to 25°C/s. The temperature section of 800 to 400°C is a temperature at which martensite transformation occurs. The martensite transformation critical cooling rate refers to a cooling rate at which a martensite single phase structure may be obtained, and more specifically, a cooling rate at which other structures than martensite do not occur in a CCT curve. When the martensite transformation critical cooling rate has the low level as described above in the temperature section of 800 to 400°C, it is easy to secure the martensite single phase structure even at a low cooling rate. When the martensite transformation critical cooling rate is less than 15°C/s, early transformation by air cooling occurs in a material transfer step, so that forming becomes difficult. When the martensite transformation critical cooling rate is more than 25°C/s, it is difficult to use a blank holding force, so that the wrinkles in a flange portion become larger.

In addition, the hot press formed part according to an example embodiment of the present disclosure may have a wrinkle wave height of the flange portion of 1 mm or less. As such, by controlling the wrinkle wave height of the flange portion into 1 mm or less, assembly with other parts may be facilitated. Meanwhile, the flange portion refers to an area fixed by an upper die and a lower holder, and spot welding may be applied to the flange portion so as to have robust connectivity with other parts. In addition, the wave height refers to a difference between the lowest point and the highest point of a wrinkle.

The hot press formed partn according to an example embodiment of the present disclosure provided as described above may be applied as a part having a deep formed depth or requiring control of material inflow. In addition, forming defects such as cracks do not occur while securing ultra-high strength, and a wrinkle wave height formed in the flange portion is also low, so that weldability improvement with other parts may also be expected.

FIG. 8 is a schematic diagram showing hot press forming equipment which may be applied to the present disclosure. Hereinafter, a method for manufacturing a hot press formed part according to an aspect of the present disclosure will be described with reference to FIG. 8.

As shown in FIG. 8, hot press forming equipment applicable to the present disclosure, that is, a mold A-100 may include: an upper die A-10; a lower punch A-20 provided in a lower center of the upper die; and a lower holder A-30 provided in a lower portion of the upper die A-10 and a side portion of the lower punch A-20. Meanwhile, a cooling channel A-12 which cools the steel material may be provided in the upper die A-10. A cooling channel A-22 which cools the steel material may be provided also in the lower die A-20. In addition, a heating heater A-32 which heats the flange portion of the steel material may be provided in the lower holder A-30.

First, the steel material is austenized. The austenizing is for forming a martensite single phase structure through hot press forming as a subsequent process by making the microstructure of the steel material into austenite. In an example embodiment of the present disclosure, the austenizing process is not particularly limited, and any common method used in the art may be used. However, as an example, the austenizing process may include heating to 850 to 950°C and then maintaining for 30 to 180 seconds.

In an example embodiment of the present disclosure, the steel material may be a steel material for hot forming described above and may have the alloy composition described above. In addition, the steel material may be obtained by the manufacturing method described above, as an example, the manufacturing method of a cold rolled steel sheet described above.

Thereafter, an austenized steel material A-200 is provided on the lower punch A-20 and the lower holder A-30. In the present disclosure, the method for providing the steel material is not particularly limited, and any common method used in the art may be used. However, the steel material is a hardenability improvement type material and may have a martensite transformation critical cooling rate in a temperature section of 500 to 200°C of 15 to 25°C/s.

Thereafter, a blank holding force (F) and heat are applied through the lower holder A-30 to heat and support the steel material A-100 between the lower holder A-30 and the upper die A-10. The blank holding force (F) and heat control material inflow so that cracks do not occur while forming the steel material into parts and serve to lower a wrinkle wave height of the flange portion.

The blank holding force (F) satisfies the following [Equation 2], and a blank holding pressure (P) may be 1 to 10 MPa. When the blank holding pressure is less than 1 MPa, a wrinkle suppression effect may not be sufficiently obtained, and when the blank holding pressure is more than 10 MPa, supercooling is performed by the upper die to cause cracks in the steel material:
$F = P \times A$
wherein P is a blank holding pressure, and A is a contact area between the lower holder and the steel material.

The heat may be applied by the heating heater A-32 provided in the lower holder A-30. For this, the minimum temperature value (Tₘᵢₙ) of the lower holder A-30 may be 300°C. Thus, cracks which may occur due to a temperature difference between an area in contact with the lower holder and an area not in contact with the lower holder may be suppressed. When the temperature of the lower holder A-30 is lower than 300°C, crack occurrence in the steel material may be caused. In addition, the maximum temperature value (Tₘₐₓ) of the lower holder may satisfy the following [Equation 3] and [Equation 4]. When the temperature of the lower holder is higher than the maximum temperature value (Tₘₐₓ), the cooling may be slower than the critical cooling rate of the material, so that a targeted material may not be secured. ${T}_{max} = {T}_{blank} - \left[\left({CR}_{min}⋅w⋅ρ⋅C\right)/h\right]$$h = a ⋅ {P}^{b}$

wherein h is a heat transfer coefficient between the steel material and the lower holder, T_{blank} is a forming temperature of the steel material, Tₘₐₓ is a maximum temperature value of the lower holder, w is a thickness of the steel material, ρ is a density of the steel material, C is a specific heat of the steel material, CRₘᵢₙ is a martensite transformation critical cooling rate, a is a heat transfer pressurization coefficient of the steel material, P is a blank holding pressure, and b is a heat transfer pressurization index of the steel material.

Herein, T_{blank} may be in a range of 650 to 850°C, w may be in a range of 0.9 to 1.8 mm, ρ may be in a range of 7.5×10⁻⁹ to 8.1×10⁻⁹ ton/mm³, C is a specific heat of material and may be in a range of 6.3×10⁸ to 8.3×10⁸ mJ/ton·K, a may be in a range of 2.0 to 2.5, and n may be in a range of 0.16 to 0.28.

Thereafter, pressure is applied through the lower punch to form the steel material and cool it. In the present disclosure, the pressure application method or the cooling method through the lower punch is not particularly limited, and any common method used in the art may be used.

Meanwhile, the temperature of the remaining portion of the mold other than the lower holder may be 300°C or lower. Thus, an area not in contact with the lower holder in the steel material may be cooled faster than the critical cooling rate after finishing forming to secure an ultra-high material. Meanwhile, in the present disclosure, the method for controlling the temperature of the remaining portion of the mold other than the lower holder is not particularly limited, and any common method used in the art may be used. However, for example, a fluid refrigerant is continuously supplied to the cooling channel A-12 provided in the upper die A-10 and the cooling channel A-22 provided in the lower punch A-20, or the fluid refrigerant is continuously brought into direct contact with the steel material, or a mord having excellent heat transfer performance may be used to ensure a targeted range of cooling rate without a separate cooling apparatus.

Hereinafter, a forming apparatus according to the fourth aspect of the present disclosure and a forming method using the same will be described.

According to an example embodiment of the present disclosure, an apparatus and a method for forming a bracket having both a curved portion and a flange simultaneously with a high-strength steel material, and forming a bracket for a battery case which is formed by the apparatus or the method and has not been conventionally formed with a high-strength steel are provided.

In an example embodiment of the present disclosure, the high-strength steel material may be the steel material for hot forming described above and may have the alloy composition described above. In addition, the material may be manufactured by the manufacturing methods described above.

FIGS. 12 and 13 illustrate the forming apparatus according to an example embodiment of the present disclosure. Specifically, FIG. 12 illustrates an exploded perspective view of the forming apparatus according to an example embodiment of the present disclosure, and FIG. 13 illustrates a side view of the forming apparatus according to an example embodiment of the present disclosure. In this example embodiment, the forming apparatus is illustrated with a focus on the exterior of the mold.

As shown in FIG. 12, the forming apparatus according to an example embodiment of the present disclosure includes: a pad B-200; a die B-300 disposed in the outside in the first direction 2 of the pad B-200; and a punch B-100 which is disposed in a lower portion of the pad B-200 and includes main body in which first to fifth punch forming portions B-120, B-130, B-140, B-150, and B-160 are formed. Though not shown in FIGS. 12 and 13, the forming apparatus according to an example embodiment of the present disclosure is a hot press forming apparatus, in which cooling channels B-170 and B-370 (see FIG. 10) in which cooling water flows are disposed inside the punch B-100 and the die B-300, thereby hardening the material through a heat treatment during forming or after forming.

The pad B-200 and the die B-300 are connected to an upper mold of the press, and the punch B-100 is connected to a lower mold of the press, so that the material is formed as the pad B-200 and the die B-300 move in a third direction 4 which is an up and down direction toward the punch B-100. Though not shown, the pad B-200 and the die B-300 are formed so that they may independently move or relative motion in an up and down direction may be performed. For example, a structure in which an elastic member is attached to an upper portion of the pad B-200, and after the pad B-200 and the die B-300 move together and forming of the pad B-200 is finished, only the die B-300 moves downward with respect to the pad B-200 by the elastic member may be applied.

The punch B-100 is formed with a structure of forming two brackets simultaneously. Therefore, two forming portions corresponding to the curved portion of the bracket are included. Specifically, the punch B-100 includes a linear first punch forming portion B-110, a curved second punch forming portion B-120 having a forming portion curve radius of curvature (Rp), a linear third punch forming portion B-130, a curved fourth forming portion B-140 having the forming portion curve radius of curvature (Rp), and a linear fifth punch forming portion B-150 consecutively along a second direction 3 perpendicular to the first direction 2 on a horizontal plane, when viewed from the first direction 2, and a support portion B-160 which supports a material before forming is disposed outside the first forming portion and the fifth forming portion B-150.

The first and fifth punch forming portions B-110 and B-150 have a structure which is tilted toward the third punch forming portion B-130 overall, the third punch forming portion B-130 has a structure parallel to the horizontal plane in the center, and the second and fourth punch forming portions B-120 and B-140 have a structure which connects the first and fifth punch forming portions B-110 and B-150 and the third punch forming portion B-130 by curving.

The first and second punch forming portions B-110 and B-120 and the fourth and fifth punch forming portions B-140 and B-150 have a symmetrical structure around the third punch forming portion B-130, and thus, one bracket is formed around the second punch forming portion B-120 and another bracket is formed around the fourth punch forming portion B-140.

The first punch forming portion B-110 includes: a first extended surface forming portion B-111 which is extended along the third direction 4 so that the flanges B-21 and B-23 (see FIG. 11) of the bracket B-20 (see FIG. 10) are formed on both sides in the first direction 2, a first main body forming portion B-113 which forms the main body B-23 (see FIG. 11) of the bracket B-20 and is disposed in a lower portion of the pad B-200, and a first curved surface forming portion B-112 having a bending radius of curvature (r) between the first extended surface forming portion B-111 and the first main body forming portion B-113.

The second punch forming portion B-120 and the third punch forming portion B-130 also include: second and third extended surface forming portions B-121 and B-131 which are extended along the third direction 4 so that the flanges B-21 and B-22 of the bracket B-20 are formed on both sides in the first direction 2, second and third main body forming portions B-123 and B-133 which form the main body B-23 of the bracket B-20 and is disposed in the lower portion of the pad B-200, and second and third curved surface forming portions B-122 and B-132 having the bending radius of curvature (r) between the second extended surface forming portion B-121 and the second main body forming portion B-113 and between the third extended surface forming portion B-131 and the third main body forming portion B-133. Herein, the third main body forming portion B-133 and the support portion B-160 may be parallel to the horizontal plane.

Since the fourth and fifth punch forming portions B-140 and B-150 have the structure symmetrical to the first and second punch forming portions B-110 and B-120, the fourth and fifth punch forming portions B-140 and B-150 also include the fourth and fifth extended surface forming portions B-141 B-151, the fourth and fifth curved surface forming portions B-142 and B-152, and the fourth and fifth main body forming portions B-143.

Meanwhile, the pad B-200 includes first to fifth pressurizing surfaces B-210, B-220, B-230, B-240, and B-250 having a shape corresponding to the first to fifth main body forming portions B-113, B-123, B-133, and B-143 of the punch B-100. The pad B-200 primarily forms a material so that it has a curved portion overall by pressurizing the material on an upper portion of the punch B-100. The pad B-200 may have a length between a length corresponding to the third main body forming portion B-133 and the third extended surface forming portion B-131 in the first direction 2.

The die B-300 is disposed on both sides in the first direction of the pad B-200 and has a structure forming the flanges B-21 and B-22. In the example embodiment, the die B-300 is disposed on both sides so that the flanges B-21 and B-22 are formed on both sides of the bracket B-20, but is not limited thereto, and may be disposed only on one side. Since the shapes of both sides of the die B-300 around the pad B-200 are symmetrical, description will focus on one side of the die B-300.

The die B-300 includes: a linear first die forming portion B-310, a curved second die forming portion B-320 having a die curve radius of curvature (Rd), a linear third die forming portion B-330, a curved fourth die forming portion B-340 having the die curve radius of curvature (Rd), and a linear fifth die forming portion B-310 so that it corresponds to the first to fifth forming portions B-110, B-120, B-130, B-140, and B-150 of the punch B-100, when viewed from the first direction 2. The first to fifth die forming portions B-310, B-320, B-330, B-340, and B-350 are connected through a vertical plane B-360.

The first and second die forming portions B-310 and B-320 and the fourth and fifth die forming portions B-340 and B-350 in the die B-300 have a symmetrical structure around the third die forming portion B-330, similarly to the punch B-100.

The first die forming portion B-310 is adjacent to the punch B-100, and includes a first die curved surface forming portion B-311 which is formed into a curved surface at a relatively close position to the punch B-100 in the first direction and a first plane forming portion B-312 which is relatively far from the punch B-100.

Likewise, the second to fifth die forming portions B-320, B-330, B-340, and B-350 include second to fifth die curved surface forming portions B-321, B-331, B-341, and B-351 and second to fifth plane forming portions B-322, B-332, B-342, and B-352. The curved surfaces of the first to fifth die curved surface forming portions B-311, B-321, B-331, B-341, and B-351 have a rising height as they are closer to the punch B-100.

In this example embodiment, the curve radius of curvature (Rd) in the second to fourth die forming portions B-320 and B-340 refers to a radius of curvature in the upper portions B-321a and B-341a closest to the punch B-100 in the second and fourth curved surface forming portions B-321 and B-341, when viewed from the first direction 2.

As seen in FIG. 13, in this example embodiment, the die B-300 is configured so that the first and fifth die forming portions B-310 and B-350 are first in contact with the material, and next the third die forming portion B-330, and finally the second and fourth die forming portions B-320 and B-340 are formed, when forming the flange, by the sequential forming, stretching/contraction is performed in a state in which the material between the second and fourth die forming portions B-320 and B-340 and the second and fourth punch forming portions B-120 and B-140 is secured, and thus, occurrence of wrinkles or tears in the forming process may be prevented.

Specifically, when the third main body forming portion B-133 and an upper portion B-331a of the third die forming portion B-330 are placed on the same plane (a), the first main body forming portion B-113 is placed above an upper portion B-311a of the first die forming portion B-310 (c), and the second main body forming portion B-123 is placed under an upper portion B-321a of the second die forming portion B-320 (b), when viewed from the first direction 2. The relationship between the fourth and fifth die forming portions B-340 and B-350 and the fourth and fifth main body forming portion B-143 and B-153 is the same.

That is, when the third die forming portion B-330 starts to perform flange forming in the material, the first die forming portion B-310 already performs flange forming, and the second die forming portion B-320 which is a curved portion does not perform forming yet.

In this example embodiment, it is configured that the length (lp) of the third main body forming portion B-133 is longer than the length (ld) of the third die forming portion B-330, and the forming portion curve radius of curvature (Rp) of the second main body forming portion B-123 is smaller than the die curve radius of curvature (Rd) of the second die forming portion B-320, thereby achieving the relationship described above.

Since the die curve radius of curvature (Rd) is formed to be larger than the forming portion curve radius of curvature (Rp), the center of the die curve radius of curvature (Rd) may be placed in the center of the second direction 3 of the third die forming portion B-330. Therefore, the centers of the die curve curvature radii of the second die forming portion B-320 and the fourth die forming portion B-340 may be placed at the same position, but are not limited thereto.

Herein, when viewed from the first direction, an angle (θ) at which extended lines of imaginary tangents intersect at both ends in the fourth punch forming portion B-143 may be 90° or more, or specifically 95 to 135°, and this is identical in the second punch forming portion B-123, of course.

Meanwhile, the forming apparatus according to an example embodiment of the present disclosure achieve the structure which is difficult to be achieved by press forming with a conventional high-strength steel of 1200 MPa or more, through hot press forming and the structure described above, and the forming portion curve radius of curvature (Rp) and the bending radius of curvature (r) may satisfy 25 mm ≤ Rp (mm) + r (mm) ≤ 30 mm.

The bracket produced by the forming apparatus may be used in the battery case as described above, and when the radius of curvature in the battery case is large, a dead space may occur, and thus, the bending radius of curvature (r) allowable for forming the flange in the battery case is substantially 10 mm or less. Meanwhile, when the bending radius of curvature (r) is less than 3 mm, forming is difficult even with a hot press forming steel of 1200 MPa or more, and even when r is 3 mm, it is determined whether forming may be performed, depending on the forming portion curve radius of curvature (Rp). This will be described again, while describing the bracket for a battery case.

FIGS. 14 to 20 relate to the method for forming according to an example embodiment of the present disclosure, in which FIG. 14 is a flow chart of the forming method according to an example embodiment of the present disclosure, FIG. 15 is a plan view of the material added to the forming apparatus according to an example embodiment of the present disclosure, FIG. 16 is a schematic perspective view illustrating a first forming process in the forming method according to an example embodiment of the present disclosure, FIGS. 17, 18a, and 18b are a schematic perspective view, other perspective view and front view illustrating a second forming process in the forming method according to an example embodiment of the present disclosure, FIG. 19 is a front view illustrating a cooling process in the forming method according to an example embodiment of the present disclosure, and FIG. 20 is a perspective view illustrating a trimming process in the forming method according to an example embodiment of the present disclosure.

Since the forming method according to another aspect of the present disclosure may be performed by the forming apparatus described above, it will be described also referring to FIG. 12.

The forming method according to an example embodiment of the present disclosure includes: a material settling process (S110) of settling a material B-400 which is longer than a punch B-100 having a forming portion in a first direction 2 in the punch B-100; a first forming process (S120) of forming the material B-400 into shapes of main body forming portions B-113, B-123, B-133, and B-143 of the punch B-100 through a pad B-200 placed on an upper portion of the punch B-100; a second forming process (S130) of forming the material so that the material B-400 follows a shape of the forming portion of the punch B-100 through a die B-300 placed on an outside of the pad B-200 in the first direction 2; a cooling process (S140) of cooling the material so as to have a martensite structure by at least one of the punch and the die; and a trimming process (S150) of cutting the formed article after cooling into a bracket shape.

The material settling process (S110) is a process of adding the material into a forming apparatus to settle the material in the punch B-100, in which the material is a steel sheet, and the material is settled in the punch B-100 in an austenite state, that is, in a state of being heated to a temperature at or higher than AC3 temperature of the material, so that a structure change may occur during or after forming. The material may be a hot press forming steel, for example, 22MnB5.

In an example embodiment of the present disclosure, the material may be a steel material for hot forming described above and may have the alloy composition described above.

In addition, the material B-400 includes a notch B-410 which is formed on both sides toward the center of the material in the center in the second direction 3 so that two brackets may be formed at once in the present disclosure. The notch B-410 prevents occurrence of cracks in an area other than the notch B-410 by narrowing a deformation range during forming.

As seen in FIG. 16, the first forming process (S120) is a process of curve forming the material B-400 through the pad B-200 after settling the material B-400, in which the material B-400 is pressurized onto the pad B-200 on the upper portion of the punch B-100 to form the material B-400.

As seen in FIGS. 17, 18a, and 18b, the second forming process (S130) is a process of forming a flange in the curve formed material through the die B-300, and is a process of pressurizing a portion which is not in contact with the pad B-200 in the first formed material B-400 by the pad B-200, with die B-300 to deform the material. Herein, as described in FIG. 13, in the second forming process (S130), the die B-300 is formed in the order of the edge portion, the center portion, and the middle portion between the center and edge portions in the second direction 3, so that the curved portion of the first formed material B-400, that is, the second and fourth punch forming portions A120 and B-140 is finally formed, thereby forming the flange in the material B-400. Herein, the shapes of the forming portions of the punch B-100 and the die B-300 are as described through FIGS. 12 and 13.

The cooling process (S140) is a process of cooling the material B-400 during or after the forming, in which the material B-400 having an austenite structure is cooled by circulating a cooling fluid through cooling channels B-170 and B-370 formed in at least one of the punch and the die, thereby transforming the austenite structure into a martensite structure, so that the material B-400 becomes a high-strength steel having a tensile strength of 1200 MPa or more. In this example embodiment, the cooling channels B-170 and B-370 are formed in both the punch B-100 and the die B-300, and if the austenite structure can be transformed into the martensite structure, the cooling channels B-170 and B-370 may be provided in either one, and, if necessary, the cooling channels B-170 and B-370 may be provided also in the pad B-200.

When the cooling process (S140) is finished, the trimming process (S150) of cutting the material B-400 which has been formed so that only the portions corresponding to two brackets remain along the cutting line B-420 is performed. Two brackets are cut around the second and fourth punch forming portions B-120 and B-140 of the punch B-100.

The forming method according to an example embodiment of the present disclosure may form the bracket having a curved portion and a flange with a high-strength steel. In addition, spring back occurring in the forming in the high-strength steel may be prevented by applying a hot press forming method, and forming errors, for example, wrinkle or thinning due to the flange forming in the curved portion may be prevented.

FIG. 21 is a perspective view of a bracket manufactured by the forming method according to an example embodiment of the present disclosure.

The bracket B-20 of FIG. 21 is curved with a forming portion curve radius of curvature (Rp) overall, while having a main body B-23 and flanges B-21 and B-22. Herein, the flanges B-21 and B-22 are connected to the main body B-23 with a curved surface B-24 curved with a bending radius of curvature (r). The surface formed with the forming portion curve radius of curvature (Rp) in the main body B-23, the flanges B-21 and B-22, and the curved surface B-24 therebetween of the bracket B-20 may be referred to as a formed surface.

FIG. 22 illustrates a distribution chart of a thickness reduction rate of a formed article manufactured by the forming method according to an example embodiment of the present disclosure (Embodiment 1-1), FIG. 23 illustrates a distribution chart of a thickness reduction rate of Comparative Illustration 1-1 manufactured by another forming method, and FIG. 24 is a thickness reduction rate distribution graph in the cross sections of the formed articles of FIGS. 22 and 23.

The distribution chart of the thickness reduction rate is a drawing showing how the thickness of the material B-400 (see FIG. 15) changed after forming, and the thickness reduction rate is obtained by subtracting the thickness of the bracket B-20 at the corresponding position from the initial thickness (tini) of the material B-400 and then dividing the value by the initial thickness (tini). When the value is positive, it means that the material becomes thinner, and when negative, it means that the material becomes thicker.

The example of FIG. 22 was manufactured by the forming apparatus of FIG. 12, and a heated material having a martensite structure was supplied to a 22MnB5 steel, the cooling rate was adjusted, and the tensile strength of the bracket was 1500 MPa. Herein, the thickness of the material was 1.2t, the bending radius of curvature (r) was 5 mm, and the forming portion curve radius of curvature (Rp) was 22 mm.

As seen in FIGS. 22 and 24, since the thickness of the main body B-23 in the bracket B-20 is no different from the initial thickness (tini), the average thickness (tav) of the main body B-23 of the bracket B-20 may be considered as the initial thickness (tini) of the material B-400, and the value obtained by subtracting the thickness at an individual position from the average thickness (tav) of the main body B-23 and then dividing the value by the average thickness (tav) may be considered as the thickness reduction rate.

Comparative Illustration 1-1 was formed by supplying a mart steel having a tensile strength of 1500 MPa as a material through the same forming apparatus.

As seen in FIG. 24, it is confirmed that when the bracket was manufactured by the forming apparatus and the forming method according to an example embodiment of the present disclosure (Embodiment 1-1), the thickness reduction rate of the portion having the maximum value of the thickness reduction rate, that is, having a minimum thickness value (tmin) was 0.2 or less, but in Comparative Illustration 1-1, the thickness reduction rate of the thinnest portion of the thickness was more than 0.2. When the thickness reduction rate is increased to more than 0.2, a height difference occurs in the flanges B-21 and B-22, so that sealability may be reduced when manufacturing a battery case.

In addition, as seen in FIG. 24, even when the bracket is curved and stretching is dominant, shrinkage occurs in a certain portion, and when buckling occurs due to the shrinkage, material damage may occur. The bracket according to the forming method according to an example embodiment of the present disclosure did not have the thickness reduction rate of -0.3 or less even at the maximum thickness (tmax) position in the curved surface, and thus, was confirmed to be stably formed even in the curved portion.

However, in Comparative Illustration 1-1, it was found that the thickness reduction rate reaching -0.8 occurred in the maximum thickness (tmax) position to cause buckling occurrence in the corresponding portion. The buckling leads to cracks and damages the structural performance of the battery case, of course, there is a possibility of water inflow into the corresponding portion, and thus, the bracket like Comparative Illustration 1-1 may not be applied to the battery case. In order to maintain sealability, it is favorable to maintain the thickness reduction rate of -0.4 or more even in the curved portion.

Meanwhile, forming is allowed only when the sum of the forming portion curve radius of curvature (Rp) and the bending radius of curvature (r) is 25 mm or more, and when primarily the bending radius of curvature (r) was less than 3 mm, it was difficult to form a bracket which may be applied to the battery case even by the forming apparatus and the forming method according to an example embodiment of the present disclosure, and even when the bending radius of curvature (r) was 3 mm and the flange was able to be formed, in the case in which the forming portion curve radius of curvature (Rp) was less than 22 mm, the forming was not performed well in the curved portion flange. Meanwhile, when the bending radius of curvature (r) and the forming portion curve radius of curvature (Rp) were increased, there was not difficulty in the forming itself, but the radius of curvature in the battery case was increased to cause a dead space, which is impractical. Therefore, it is preferred that the bracket applied the battery case has the sum of the forming portion curve radius of curvature (Rp) and the bending radius of curvature (r) of 30 mm or less.

In addition, an angle (θ) at which the extended lines of the imaginary tangents intersect at both ends of the formed surface in the bracket B-20 may be 95 to 135°, and when the angle (θ) was less than 95°, the forming was not performed well even when the conditions of the forming portion curve radius of curvature (Rp) and the bending radius of curvature (r) were satisfied. When the angle (θ) is more than 135°, the battery case should be composed of angles more than an octagon, and thus, a dead space which is not occupied by battery cells having a roughly rectangular shape occurs, which is impractical.

Meanwhile, FIG. 25 is a side view illustrating the forming method of Comparative Illustration 1-2, and FIG. 26 is a perspective view of the formed article manufactured by the forming method of Comparative Illustration 1-2.

Though the order of the forming method of FIG. 25 is identical to the order of the forming method of the present disclosure, the flange forming was not performed in the order of the edge, the center, and the curved portion in the second direction 3 in the second forming process (S130), but forming was performed with the die B-300 composed so that the forming was performed in the order of the center, the curved portion, and the edge. In Comparative Illustration 1-2, the die B-300 is composed so that the center has the lowest upper portion B-301a position, and sequential forming is performed toward the outside.

When the forming is performed as such, even in the case of identically applying a hot press forming process, as seen in FIG. 26, a folded area B occurs, thereby manufacturing a bracket which may not be used as a battery case.

Hereinabove, the example embodiments of the present disclosure were mainly described, but the present disclosure is not limited thereto, and may be variously modified and carried out, of course.

Hereinafter, the hot press formed part according to the fifth aspect of the present disclosure will be described.

FIG. 27 is a perspective view of the formed part according to an example embodiment of the present disclosure, and FIG. 28 is a front view of the formed part according to an example embodiment of the present disclosure.

The hot press formed part according to an example embodiment of the present disclosure includes: a first wall C-110 extended in a first direction (Y direction), a second wall C-120 extended in a direction intersecting the first wall C-110, wherein a curvature portion C-160 is formed between the first wall C-110 and the second wall C-120, an angle between an arbitrary line perpendicular to the first direction (line parallel to the Z direction) and the second wall C-120 is 0° or more and 5° or less, and the first wall C-110, the second wall C-120, and the curvature portion C-160 are integrally formed.

The hot press formed part according to an example embodiment of the present disclosure includes the first wall C-110, the second wall C-120, and the curvature portion C-160 placed between the first wall C-110 and the second wall C-120. the first wall C-110, the curvature portion C-160, and the second wall C-120 are integrally formed so as to extend sequentially.

The hot press formed part is characterized by being integrally formed by including the first wall C-110 formed to be parallel in the first direction, the curvature portion C-160 curved from the first wall C-110, and the second wall C-120 connected to one end of the curvature portion C-160.

When an arbitrary line perpendicular to the first direction is assumed, the second wall C-120 may have an angle with the arbitrary line of 0° or more and 5° or less.

Many parts using a high-strength steel are being produced according to the demand for vehicle weight reduction and safety improvement, and it is difficult to use the high-strength steel in the production of parts having a small radius of curvature due to poor bendability.

The hot press forming method is a working method of heating a blank, forming the heated blank into a desired shape through press forming, and cooling it with a mold closed to manufacture a high-strength formed part. In the hot press forming method as such, when the hot press forming method which is formed at a high temperature is used, even parts having a small radius of curvature may be formed without cracking due to excellent characteristics of an elongation of 50% or more at a high temperature at which forming is performed, and thus, the shape of formed parts which may not be secured with cold ultra-high strength may be secured.

An example embodiment of the present disclosure relates to a formed part C-10 which is integrally formed by including the first wall C-110, the curvature portion C-160, and the second wall C-120 through the hot press forming method, wherein the second wall C-120 has an angle with the arbitrary line of 0° or more and 5° or less, which is smaller than the conventional parts. Therefore, the first wall C-110 and the second wall C-120 have a shape close to a right angle and may have efficiency in use of the space surrounded by the first wall C-110 and the second wall C-120.

According to an example embodiment of the present disclosure, the first wall C-110, the second wall C-120, and the curvature portion C-160 may be integrally formed by working a sheet material.

The first wall C-110, the curvature portion C-160, and the second wall C-120may be integrally formed according to the hot press forming method, using a single sheet material or a sheet material in which a plurality of sheet materials are combined in the thickness direction, as a blank. Since they are integrally formed by hot press, working is convenient, and the formed part C-10 having a relatively high tensile strength may be manufactured while problems in working in the joint portion such as a weld, damage due to stress concentration, or the like is prevented.

In an example embodiment of the present disclosure, the sheet material may be a steel material for hot forming described above and may have the alloy composition described above.

According to an example embodiment of the present disclosure, the radius of curvature (r) of the curvature portion C-160 may be 0.5 mm or more, and a limit bending (r/t) which is a ratio between the thickness (t) and the radius of curvature (r) of the sheet material may be less than 2.5.

The ratio (r/t) between the thickness (t) and the radius of curvature (r) of the sheet material before working generally depends on the limit bending value of a raw material. The limit bending may be a numerical value expressing a maximum radius of curvature at which lag does not occur as compared to the material thickness. Since it is common that the thickness (t) of the sheet material is predetermined before working, when the radius of curvature is decreased to be smaller than the ratio (r/t) which may be formed in the sheet material, cracks occur on the formed part C-10.

According to an example embodiment of the present disclosure, the ratio (r/t) between the thickness (t) and the radius of curvature (r) of the sheet material may be less than 2.5. As compared to this, the limit bending of a conventional ultra-high strength material of a tensile strength of a 1500 MPa grade is known as 2.5 or more. For example, it means that the minimum radius of curvature of the part which may be formed with an ultra-high strength of a 1500 MPa grade of a material having a thickness of 1.0 mm is 2.5 mm or more. However, according to the present disclosure, even when it is formed with ultra-high strength, it may have the ratio (r/t) value of less than 2.5, and thus, a product having the ratio (r/t) of less than 2.5 may be formed even with the ultra-high material of a tensile strength of a 1500 MPa grade. Therefore, the formed part according to an example embodiment of the present disclosure may be a part having excellent formability and a high space utilization. According to an example embodiment of the present disclosure, a third wall C-130 and a fourth wall C-140 parallel to the first direction and a fifth wall C-150 connected to the third wall C-130 and the fourth wall C-140 are included, the third wall C-130 is extended from the second wall C-120, and the first wall C-110 to the fifth wall C-150 may be integrally formed.

According to the hot press forming process, hat shapes having a plurality of wall surfaces may be formed at once, and thus, formability is excellent.

As an example, the third wall C-130 and the fourth wall C-140 parallel to the first direction may be formed, and the first wall C-110 and the fourth wall C-140 may have the same height in the direction perpendicular to the first direction, but the present disclosure is not limited thereto. Further, the third wall C-130 may have different heights. The fifth wall may be placed between the third wall C-130 and the fourth wall C-140, the second wall C-120 and the third wall C-130 may be connected to the first connection portion C-170, the third wall C-130 and the fifth wall C-150 may be connected to the second connection portion C-180, and the fifth wall C-150 and the fourth wall C-140 may be connected to the third connection portion C-190. Therefore, the first wall to the fifth wall C-150, the curvature portion C-160, and the first connection portion C-170 to the third connection portion C-190 may be integrally formed by working a sheet material.

Herein, the first connection portion C-170 and the third connection portion C-190 may be formed into a shape having a radius of curvature as in the curvature portion C-160, in which the radius of curvature may have all of the characteristics of the curvature portion C-160 of the first wall C-110 and the second wall C-120. However, the present disclosure is not limited to the shape.

According to an example embodiment of the present disclosure, the formed part may have the tensile strength of 1300 to 2100 MPa.

The tensile strength referred to as ultra-high strength may be generally about 1500 MPa. According to the present disclosure, a formed part having a tensile strength which may be considered as high strength or ultra-high strength of about 1300 to 2100 MPa may be manufactured. Since the formability becomes better due to the hot press forming, the formed part according to an example embodiment of the present disclosure is integrally manufactured and may be manufactured to have a tensile strength of ultra-high strength while forming parts having a relatively small radius of curvature.

In addition, the parts having a small radius of curvature may be formed even with a steel for hot press forming of a 1800 MPa and 2000 MPa grade, when excellent formability at a high temperature is utilized. Therefore, according to the present disclosure, even formed parts having a small radius of curvature having a tensile strength of 1700 MPa to 1900 MPa, furthermore, 1900 MPa to 2100 MPa may be manufactured.

In addition, the microstructure forming the formed part C-10 may have martensite at an area fraction of 98% or more. Since most of the area fraction of the formed part C-10 according to the present disclosure is occupied by martensite which is a hard phase having high strength, it may form a tensile strength of an ultra-high strength grade as described above.

As an example, the formed part may be formed by martensite at an area fraction of 98% or more and include a small amount of other phases such as ferrite or bainite.

According to an example embodiment of the present disclosure, a third wall C-130 which is parallel to the first direction and is connected to the second wall C-120 may be further included, and when a length from the first wall C-110 to the third wall C-130, which is perpendicular to the first direction is defined as a wall portion height (hw), and an angle between an arbitrary line perpendicular to the first direction and the second wall C-120 is defined as a wall portion angle (θw), the following Relation 3 may be satisfied:

$hw \leq 13.4 * θw + 182.4$
wherein the unit of hw is mm, the unit of θw is degree, and calculation is performed by making the left and right sides dimensionless.

The formed part which satisfies Relation 3 and worked by hot press forming may be manufactured with excellent quality without defects such as cracks.

Referring to the following Table 1, it was found that when the Relation is satisfied, formability is excellent.

**[Table 1]**

| | θw (°) | Hw (mm) | Calculated value of right side | Whether Relation 3 was satisfied | Formability |
|---|---|---|---|---|---|
| Inventive Illustration 2-1 | 0 | 180 | 182.4 | Satisfied | Good |
| Inventive Illustration 2-2 | 1 | 190 | 195.8 | Satisfied | Good |
| Inventive Illustration 2-3 | 3 | 220 | 222.6 | Satisfied | Good |
| Inventive Illustration 2-4 | 5 | 240 | 249.4 | Satisfied | Good |
| Comparative illustration 2-1 | 0 | 190 | 182.4 | Unsatisfied | Poor |
| Comparative illustration 2-2 | 1 | 200 | 195.8 | Unsatisfied | Poor |
| Comparative illustration 2-3 | 3 | 230 | 222.6 | Unsatisfied | Poor |
| Comparative illustration 2-4 | 5 | 260 | 249.4 | Unsatisfied | Poor |

Comparative Illustrations 2-1 to 2-4 were all formed identically to Inventive Illustrations 2-1 to 2-4, respectively, except the wall portion height indicated above. However, as a result of forming the comparative examples had problems such as poor formability such as cracks.

FIG. 29a is a drawing which was interpreted identically to the conditions of Inventive Example 1, and FIG. 29b is a drawing which was interpreted as the conditions of Comparative Illustration 2-1. When FIG. 29a and FIG. 29b were compared, it was found that in Comparative Illustration 2-1, cracks marked in red occurred in an upper portion of the second wall C-120 or the fifth wall C-150, and some portions in yellow were interpreted as portions at risk of crack occurrence.

FIG. 30a is a drawing which was interpreted identically to the conditions of Inventive Illustration 2-3, and FIG. 30b is a drawing which was interpreted as the conditions of Comparative Illustration 2-3. When FIG. 30a and FIG. 30b were compared, it was found that in Comparative Illustration 2-3, cracks marked in red occurred in a lower portion of the second wall C-120 or the fifth wall C-150, and some portions in yellow were interpreted as portions at risk of crack occurrence. In comparison, Inventive Illustration 2-3 had some portions at risk of crack occurrence marked in yellow, but no crack occurrence.

Hereinafter, the battery pack module which is another aspect of the present disclosure will be described.

The following battery pack module includes the formed parts described above, and the description of the formed parts cites the above.

FIG. 31 is a drawing illustrating the battery pack module according to an example embodiment of the present disclosure, and FIG. 32 is a drawing for showing a space utilization when the battery pack module is placed, by expressing the cross section of a portion of the battery pack module, in which (a) shows the case in which the radius of curvature of the hot press formed part is small, and (b) shows the case in which the radius of curvature is larger than the case (a).

The battery pack module C-11 according to an example embodiment of the present disclosure includes: a battery case C-20 formed around a battery pack, a base C-30 which is placed in a lower portion of the battery case C-20 and is connected to the battery case C-20 to form a space where the battery pack is placed, and a hot press formed part C-10 which is placed across an inside of the battery case C-20 and is connected to the battery case C-20 and the base C-30.

The battery case C-20 has a configuration formed around the side surfaces of the battery pack, and the base C-30 has a common sheet material or, if necessary, bends or grooves and has a configuration in which the battery pack is settled.

As an example, in order to prevent collision, a reinforcing member C-40 attached to the outer surface of the battery case C-20 may be further included.

As an example, the hot press formed part C-10 reinforces rigidity for preparing for impact from collision of a battery frame as a cross member and may be placed inside the battery case C-20.

As an example, the hot press formed part C-10 may be disposed in multiples at regular intervals in the battery case C-20.

The battery pack is placed in a space formed between the base C-30, the battery case C-20, and the cross member, and the battery pack module C-1 is for stably placing the battery in a vehicle body by including the battery pack.

The formed part having a radius of curvature smaller than that of the conventional parts and high tensile strength is placed in the battery pack to increase the rigidity of the battery pack module C-1 itself, thereby preventing fire and the like due to battery damage by impact.

In addition, since generally the cross member is provided in multiples in the battery case C-20, the size of the battery pack may be increased according to the benefits of an increased space utilization, and thus, when the battery pack module C-1 has the same volume, an effect of increasing a battery capacity is provided.

As an example of being used as the cross member, when the radius of curvature (r2) in a lower end portion of the hot press formed part C-10b of Embodiment 2-2 in FIG. 32B is larger than the radius of curvature (r1) in the lower end portion of the hot press formed part C-10a of Embodiment 2-1 in FIG. 32A, it may be recognized by comparing gaps which are remaining spaces after placing the battery pack b. Since the gap g2 of FIG. 32B is larger than the gap g1 of FIG. 32A to increase the radius of curvature (r), the space which is not available for loading of the battery pack b is formed to be larger.

Further, it is recognized that the fact that space utilization is increased with the decreasing radius of curvature (r) has greater utility when a plurality of cross members are mounted in the same battery pack module C-1.

Hereinafter, the hot press formed part according to the sixth aspect of the present disclosure will be described.

FIG. 33 is a perspective view illustrating a press formed part according to an example embodiment of the present disclosure. FIG. 34 is a perspective view illustrating a press formed part according to another example embodiment of the present disclosure. In FIG. 35, (a) is a graph showing a relationship between a predetermined length and a predetermined height of the press formed part according to an example embodiment of the present disclosure, and (b) is a graph showing a relationship between a predetermined length and a predetermined height of the press formed part according to another example embodiment of the present disclosure. Further, in FIG. 36, (a) illustrates an example showing a deformation force applied to the press formed part manufactured using a conventional manufacturing method, and (b) illustrates an example showing a deformation force applied to the press formed part manufactured using the manufacturing method according to the example embodiments of the present disclosure.

Referring to FIGS. 33 and 34, the press formed parts D-10 and D-10' according to example embodiments of the present disclosure may be manufactured by performing press forming working on a metal sheet. Herein, the hot press forming method may be used in the manufacture of press formed parts D-10 and D-10'.

The press formed parts D-10 and D-10' may include a flat plate portion D-110 which is not press formed to have a flat shape and a deformation portion D-120 which has a convex shape toward one direction by press forming. Herein, the deformation portion D-120 may be formed in multiples. In this case, the flat plate portion D-110 may be disposed between a plurality of deformation portions D-120.

The deformation portion D-120 may have a convex shape protruding upward (+Z), based on the drawing. Herein, the deformation portion D-120 may include a top plate portion D-121, a vertical wall portion D-122, and a boundary portion D-123.

The top plate portion D-121 may be an upper end portion of the deformation portion D-120 extending in the first direction. Herein, the first direction may be, for example, a direction parallel to a longitudinal direction Y of the press formed parts D-10 and D-10'.

The vertical wall portion D-122 may be a side wall portion of the deformation portion D-120 extending in the second direction. Herein, the second direction may be a direction different from the first direction described above. As an example, the second direction may be a direction inclined toward the first direction at a certain angle. As another example, the second direction is a direction perpendicular to the first direction and may be parallel to the up and down direction Z in the drawing. Meanwhile, the up and down direction Z may be parallel to the height direction of the deformation portion D-120.

The vertical wall portion D-122 may be continuous with the top plate portion D-121. More specifically, the vertical wall portion D-122 may be disposed so that the upper end is continuous with one side end of the top plate portion D-121. The vertical wall portion D-122 may be provided in a pair. A pair of vertical wall portions D-122 are disposed to be continuous with both side ends of the top plate portion D-121, respectively to form both side wall portions of the deformation portion D-120.

The portion D-121a (hereinafter, referred to as a shoulder portion) where the side end of the top plate portion D-121 and the upper end of the vertical wall portion D-122 are connected may have a round shape having a first radius of curvature. Herein, the shoulder portion D-121a may be convexly curved outward from the deformation portion D-120.

The boundary portion D-123 may be a boundary between the deformation portion D-120 and the flat plate portion D-110 which are continuous along the longitudinal direction Y of the press formed parts D-10 and D-10'. One end of the boundary portion D-123 may be continuous with the lower end of the vertical wall portion D-122, and the other end of the boundary portion D-123 may be continuous with one end of the flat plate portion D-110. Herein, the other end of the flat plate portion D-110 may be continuous with the boundary portion D-123 provided in another deformation portion D-120. The boundary portion D-123 is provided in a pair and may be disposed so that it is continuous with each of the lower ends of a pair of vertical wall portions D-122.

The boundary portion D-123 may have a round shape with a second radius of curvature. The boundary portion D-123 may be concavely curved inward from the deformation portion D-120. Herein, the second radius of curvature may be identical or similar to the first radius of curvature.

As described above, the deformation portion D-120 may have a form in which the boundary portion D-123, the vertical wall portion D-122, the top plate portion D-121, the vertical wall portion D-122, and the boundary portion D-123 are sequentially continuous along the longitudinal direction Y. Accordingly, the deformation portion D-120 may have a hat shape or a shape similar thereto.

The deformation portion D-120 as described above may be provided in multiples. More specifically, at least three deformation portions D-120 may be provided. In this case, the flat plate portion D-110 may be disposed between adjacent two deformation portions D-120 among a plurality of deformation portions D-120. Herein, the adjacent two deformation portions D-120 may be continuous by the flat plate portion D-110 placed in the center.

Accordingly, the press formed parts D-10 and D-10' may have a form in which 3 or more deformation portions D-120 and a plurality of flat plate portions D-110 may be disposed alternately in a row along the longitudinal direction Y. Herein, the flat plate portion D-110 may be disposed in both outer sides of the press formed parts D-10 and D-10' based on the longitudinal direction Y, but is not limited thereto.

The deformation portion D-120 may be formed at a predetermined height (h). Herein, the predetermined height (h) is a height of the deformation portion D-120, and means a length from the lower surface of the flat plate portion D-110 to the upper surface of the top plate portion D-121.

The adjacent two deformation portion D-120 may be spaced apart by a predetermined length (w) along the longitudinal direction Y. Herein, the predetermined length (w) may refer to a length of the flat plate portion D-110 measured based on the longitudinal direction Y. Herein, the predetermined length (w) may be measured based on the flat plate portion D-110 disposed between the adjacent two deformation portions D-120.

As shown in FIG. 33, the press formed part D-10 according to an example embodiment of the present disclosure (hereinafter, referred to as Embodiment 3-1) may include three deformation portions D-120. Accordingly, the press formed partn D-10 of Embodiment 3-1 may include at least two flat plate portions D-110 disposed between the three deformation portions D-120.

As shown in FIG. 34, the press formed part D-10' according to another example embodiment of the present disclosure (hereinafter, referred to as Embodiment 3-2) may include four or more deformation portions D-120. Accordingly, the press formed part D-10 of Example 1 may include at least three flat plate portions D-110 disposed between the four deformation portions D-120.

Meanwhile, only the case in which the press formed part D-10' is provided with four deformation portion D-120 is illustrated in the drawing, but the present disclosure is not limited thereto. Though not illustrated in the drawing, as another example, 5 or more deformation portions D-120 may be formed in the press formed part D-10', in which the upper limit of the number of the deformation portions D-120 is not limited.

Referring to FIGS. 35 and 36, in the conventional hot press forming method, the deformation portion D-120 is first formed, and then a separate flat plate type metal sheet is attached to the lower end of the deformation portion D-120 after forming. In this case, as the number of the deformation portions D-120 to be formed is increased, a force (deformation force, stress) is concentrated on the vertical wall portion D-122 connected to the flat plate type metal sheet and its periphery (A1 and B1 of FIG. 36A) in the manufacturing process, as illustratively shown in (a) of FIG. 36. Thus, cracks and the like occur in the deformation portion D-120 of the press formed part to cause damage. In order to prevent this, a distance between the connected deformation portions D-120 should be increased, and since the size of the manufactured press formed parts D-10 and D-10' has to be limited, the number of deformation portions D-120 which may be included therein is also limited.

Thus, in an example embodiment of the present disclosure, press formed parts D-10 and D-10' which may prevent damage in the deformation portion D-120 due to the hot press forming are intended to be provided, using a relationship between the height (predetermined height, h) of the deformation portion D-120 and a separation distance (predetermined length, w) between adjacent two deformation portions D-120. Herein, "the relationship between the predetermined height (h) and the predetermined length (w)" may be determined based on the number of the deformation portions D-120 formed in the press formed parts D-10 and D-10'.

In the press formed parts D-10 according to Embodiment 3-1 of the present disclosure, three deformation portion D-120 is formed, and thus, the relationship between "the predetermined height (h)" of the deformation portion D-120 and "the predetermined length (w)" where the adjacent two deformation portions D-120 are separated may be defined by the following Equation (1):
${w}_{min} \leq w \leq 114.85 {e}^{0.0455 h}$
wherein w is a predetermined length of Embodiment 3-1, and h is a predetermined height of Embodiment 3-1. Further, wₘᵢₙ may refer to a minimum value (that is, a minimum spacing) of the predetermined length (w) of Embodiment 3-1.

As illustrated in the graph of (a) of FIG. 35 and (b) of FIG. 36, when it is designed that the distance (predetermined length, w) between three deformation portions D-120 included in the press formed parts D-10 separated from each other satisfies Equation (1), occurrence of damage such as cracks in the deformation portion D-120 and the surrounding portion (A2 and B2 in (b) of FIG. 36) in the hot press forming process may be significantly decreased. Herein, the method for manufacturing a press formed part D-10 according to Embodiment 3-1 will be described in detail in the following.

In addition, in the press formed parts D-10 according to Embodiment 3-2 of the present disclosure, 4 or more deformation portion D-120 is formed, and thus, the relationship between "the predetermined height (h)" of the deformation portion D-120 and "the predetermined length (w)" where the adjacent two deformation portions D-120 are separated may be defined by the following Equation (2):${w}_{min} \leq w \leq 46 {. 309 e}^{0.105 h}$
wherein w is a predetermined length of Embodiment 3-2, and h is a predetermined height of Embodiment 3-2. Further, wₘᵢₙ may refer to a minimum value of the predetermined length of Embodiment 3-2.

As illustrated in the graph of (b) of FIG. 35 and (b) of FIG. 36, when it is designed that the distance (predetermined length, w) between three deformation portions D-120 included in the press formed part D-10 separated from each other satisfies Equation (1), occurrence of damage such as cracks in the deformation portion D-120 and the surrounding portion (A2 and B2 in (b) of FIG. 36) in the hot press forming process may be significantly decreased. Herein, the method for manufacturing a press formed part D-10 according to Embodiment 3-1 will be described in detail in the following.

Meanwhile, in Embodiments 3-1 and 3-2 described above, the predetermined length (w) may be 20 mm or more. That is, a minimum spacing (wₘᵢₙ) of the two deformation portions D-120 adjacent to each other may be 20 mm. This may be a minimum spacing required for securing a space for disposing a cooling hole (not shown) between first pressurizing portions D-210 provided in the molds D-200 and D-400, and/or between the second pressurizing portion D-410 and the intermediate pressurizing portion D-300, in the manufacturing apparatus D-20 and D-20' of the press formed parts D-10 and D-10' described later.

FIG. 37 is a flow chart showing the method for manufacturing a press formed part according to an example embodiment of the present disclosure. FIG. 38 schematically illustrates a first process of manufacturing the press formed part of FIG. 33. FIG. 39 schematically illustrates a second process of manufacturing the press formed part of FIG. 33. FIG. 40 schematically illustrates a third process of manufacturing the press formed part of FIG. 33. Further, FIG. 41 schematically illustrates a fourth process of manufacturing the press formed part of FIG. 33.

Referring to FIGS. 37 to 41, the manufacturing apparatus D-20 for manufacturing the press formed part D-10 according to Embodiment 3-1 may include a first mold D-200, an intermediate pressurizing portion D-300, and a second mold D-400. In this case, one intermediate pressurizing portion D-300 may be provided. Herein, the first mold D-200 may be an upper mold, and the second mold D-400 may be a lower mold, based on the up and down direction Z.

The first mold D-200 and the second mold D-400 may be disposed to face each other along the pressurizing direction-Z. The first mold D-200 may be disposed on the upper side of the second mold D-400. Herein, the first mold D-200 may be installed in an elevatable and drivable upper support (not shown). Thus, the first mold D-200 may descend toward the second mold D-400 or rise away from the second mold D-400. Further, the second mold D-400 may be disposed, for example, on a lower support (not shown) which is fixedly installed on the floor surface of a building in which the manufacturing apparatus D-20 is installed.

The first mold D-200 may be provided with the first pressurizing portion D-210. The first pressurizing portion D-210 may pressurize the upper surface of a metal sheet during press forming. Herein, the metal sheet may be a material used for manufacturing the press formed part D-10. The metal sheet before press forming may have, for example, an upper surface and a lower surface having a flat shape. Herein, the first pressurizing portion D-210 may be configured to have the shape and size corresponding to the "upper surface of the deformation portion D-120 of the press formed part D-10" described above.

The manufacturing apparatus D-20 is for manufacturing a press formed part D-10 of Embodiment 3-1, and three first pressurizing portions D-210 may be provided. Herein, the three first pressurizing portion D-210 may be separated from each other by a first distance. The first distance may be the same as the predetermined length (w) described above. In addition, the first mold D-200 may be provided with the first plane portion D-220. The first plane portion D-220 may be disposed between the adjacent two first pressurizing portions D-210. The first plane portion D-220 may be extended parallel to the longitudinal direction Y between two first pressurizing portions D-210 and connect the first pressurizing portions D-210. As described above, since three first pressurizing portions D-210 are provided, at least two first plane portions D-220 may be provided.

Accordingly, the first mold D-220 may have a form in which three first pressurizing portions D-210 are separated by the first distance (that is, the predetermined length, W) along the longitudinal direction Y, the first plane portions C-220 are disposed between them to connect the first pressurizing portions D-210.

The second mold D-400 may be provided with the second pressurizing portion D-410 and the second plane portion D-420a. Herein, the second pressurizing portion D-410 may be formed into a shape and a size corresponding to the lower surface of the press formed part D-10.

Unlike the first mold D-200, the second mold D-400 may be provided with only two second pressurizing portions D-410. In this case, the two second pressurizing portions D-410 may be disposed to be symmetrical to the two first pressurizing portions D-210 placed on both sides among the three first pressurizing portions D-210, along the longitudinal direction Y. Accordingly, in the second mold D-400, there is no second pressurizing portion D-410 in an area (hereinafter, center area) facing the first pressurizing portion D-210 in the center among the three first pressurizing portions D-210.

Accordingly, the second mold D-400 may be a single structure having a shape connected by the two second pressurizing portions D-410 and the second plane portion D-420a disposed therebetween. Herein, the plane portion D-420a may be provided with a penetration portion D-420aa. An intermediate pressurizing portion D-300 may be inserted into the penetration portion C-420aa, during press forming on an outer area of the metal sheet D-10A. The penetration portion D-420aa may be formed by penetrating one portion of the plane portion D-420a along the up and down direction Z. The penetration portion D-420aa may have a form having the crosssectional shape and area corresponding to the shape and size of the intermediate pressurizing portion D-300. In addition, a plane portion 2-2 D-420b may be further provided, respectively, on both sides of the first pressurizing portions D-210.

The intermediate pressurizing portion D-300 may be disposed between the first mold D-200 and the second mold D-400. As shown in FIG. 38, the metal sheet D-10A which is the subject to be press forming may be disposed in the lower side of the first mold D-200. In this case, the intermediate pressurizing portion D-300 is placed between the metal sheet D-10A and the second mold D-400, and when the first mold D-200 descends, a portion of the lower surface of the metal sheet D-10A may be pressurized. The intermediate pressurizing portion D-300 may be a pad for bend working by pressurizing the lower surface of the metal sheet D-10A.

The intermediate pressurizing portion D-300 may be placed directly on the center area described above of the second mold D-400. Herein, the intermediate pressurizing portion D-300 may have the same shape as the second pressurizing portion D-410. That is, the intermediate pressurizing portion D-300 may have the shape and size corresponding to the lower surface of the press formed part D-10. The intermediate pressurizing portion D-300 pressurizes the metal sheet D-10A up and down, together with the first pressurizing portion D-210 in the center among the three first pressurizing portions D-210, during press forming, thereby forming the deformation portion D-120 placed in the center.

The intermediate pressurizing portion D-300 may be configured to be elevatable. Thus, the intermediate pressurizing portion D-300 may descend along the pressurizing direction-Z, during press forming. In addition, the intermediate pressurizing portion D-300 may rise in the opposite direction Z to the pressurizing direction, after completing press forming. The rise of the intermediate pressurizing portion D-300 as such may be implemented by an elastic member (not shown) installed in the intermediate pressurizing portion D-300.

The "method for manufacturing a press formed part D-10 according to Embodiment 3-1" using the manufacturing apparatus D-20 may be as follows.

First, a metal sheet D-10A may be supplied to the manufacturing apparatus D-20 (S100). Before starting the press forming, the metal sheet D-10A may be disposed at a position between the first mold D-200 and the intermediate pressurizing portion D-300 (hereinafter, referred to as a working position), as shown in FIG. 38. Meanwhile, the metal sheet D-10A may be supplied to the manufacturing apparatus D-20, in a state of being heated by a separate heating apparatus (not shown).

As an example, the metal sheet D-10A is in the working position, the upper surface of the metal sheet D-10A may be in a state of being disposed so that it is in contact with the lower surface of the first mold D-200 or only a minor gap exists. Herein, the second mold D-400 may be in a state of being disposed to be symmetrical to the first mold D-200, with the metal sheet D-10A and the intermediate pressurizing portion D-300 interposed therebetween.

In addition, when the metal sheet D-10A is in a state of being disposed in the working position (that is, before starting press forming), the intermediate pressurizing portion D-300 may be disposed in the upper side of the second mold D-400. Accordingly, there may be a height difference (hi) between the intermediate pressurizing portion D-300 and the second pressurizing portion D-410. Herein, the height difference (hi) described above may refer to a distance from the upper surface of the second pressurizing portion D-410 to the upper surface of the intermediate pressurizing portion D-300. In this case, the height difference (hi) between the intermediate pressurizing portion D-300 and the second pressurizing portion D-410 may be smaller than the "predetermined height (h)" which is the height of the press formed part D-10. Herein, the height difference (hi) may be 65% or more of the predetermined height (h). When the manufacturing apparatus D-20 is configured to have the height difference (hi) as such, occurrence of damage such as cracks in the deformation portion D-120 formed by press forming may be significantly decreased.

Next, first press forming of the metal sheet D-10A may be performed by the first mold D-200 and the intermediate pressurizing portion D-300 (S200). As shown in FIG. 39, the first mold D-200 may descend along the pressurizing direction -Z and pressurize the upper surface of the metal sheet D-10A. In this case, the first mold D-200 may descend to the position where the lower surface of the metal sheet D-10A is not in contact with the second mold D-400. Herein, since the intermediate pressurizing portion D-300 is disposed to be higher than the second pressurizing portion D-410 by the height difference (hi) described above, only the intermediate pressurizing portion D-300 may be introduced into the first pressurizing portion D-210 and pressurize the center area of the metal sheet D-10A. Accordingly, only the center area of the metal sheet D-10A may be pressed in the up and down direction by the first pressurizing portion D-210 among the three first pressurizing portions D-210 and the intermediate pressurizing portion D-300. Thus, only the center area of the metal sheet D-10A is bend-worked, thereby forming one deformation portion D-120.

Next, second press forming of the metal sheet D-10A may be performed by the first mold D-200 and the second mold D-400 (S300). After performing the first press forming in S200, the first mold D-200 may further descend along the pressurizing direction-Z, as shown in FIG. 40. In this process, the intermediate pressurizing portion D-300 may descend together with the first mold D-200, in a state of being introduced into the first pressurizing portion D-210 in the center together with the center area of the metal sheet D-10A. Accordingly, the outer area of the metal sheet D-10A may be in contact with the upper surface of the two second pressurizing portions D-410.

Thereafter, as the first mold C-200 continues to descend, the second pressurizing portion D-410 is introduced to the first pressurizing portion D-210 and may pressurize the both outer areas of the metal sheet D-10A. In this process, the intermediate pressurizing portion D-300 may be housed in the penetration portion D-420aa of the second mold D-400. The both outer areas of the metal sheet D-10A may be pressed in the up and down direction simultaneously by the two outer first pressurizing portions D-210 and the two outer second pressurizing portions D-410. Thus, the both outer areas of the metal sheet D-10A is bend-worked, thereby further forming two deformation portions D-120.

Next, the first mold D-200 and the intermediate pressurizing portion D-300 may return to its original position (S400). After the "stepwise press forming" in S200 and S300 as described above, the first mold D-200 may rise in the opposite direction +Z to the pressurizing direction -Z, as shown in FIG. 9. In this process, the deformation portions D-120 may be separated from the first pressurizing portions D-210. In addition, the intermediate pressurizing portion D-300 may be separated from the deformation portion D-120 in the center and return to its original position. Thus, the manufacture of the press formed part D-10 in the form in which the three deformation portions D-120 having a predetermined height (h) are separated from each other by the predetermined length (w) may be completed.

Next, the press formed part D-10 after manufacture may be discharged (S500). The press formed part D-10 may be transported for the next working or manufacturing process, after being discharged from the manufacturing apparatus D-20. Thereafter, the manufacturing method described above may be repeatedly performed, by supplying the next metal sheet D-10A.

FIG. 42 schematically illustrates a first process of manufacturing the press formed part of FIG. 34. FIG. 43 schematically illustrates a second process of manufacturing the press formed part of FIG. 34. FIG. 44 schematically illustrates a third process of manufacturing the press formed part of FIG. 34. Further, FIG. 45 schematically illustrates a fourth process of manufacturing the press formed part of FIG. 34.

Referring to FIGS. 37 and 42 to 45, the press formed part D-10 according to Embodiment 3-2 may be manufactured by the manufacturing method as described below. The manufacturing apparatus D-20' for a press formed part may include a first mold D-200, an intermediate pressurizing portion D-300, and a second mold D-400. Herein, at least two intermediate pressurizing portions D-300 may be provided. In this case, since most of the characteristics of the first mold D-200, the intermediate pressurizing portion D-300, and the second mold D-400 are identical or similar to the case of Embodiment 3-1 described above, duplicate description will be omitted.

Since the press formed part D-10' according to Embodiment 3-2 is provided with 4 or more deformation portions D-120, the first mold D-200 may be provided with 4 or more first pressurizing portions D-210. Hereinafter, for convenience of description, description will focus on the case in which four first pressurizing portions D-210 are provided and separated from each other by the predetermined length (w). In this case, two first pressurizing portions D-210 are disposed in the center area of the first mold D-200, and the first pressurizing portions D-210 may be disposed one by one on both sides around them.

Two second pressurizing portions D-410 may be provided in the second mold D-400. Herein, the two second pressurizing portions D-410 may be disposed to face the two first pressurizing portions D-210 which are disposed, respectively on both sides of the first mold D-200.

When four first pressurizing portions D-210 are provided, two intermediate pressurizing portions D-300 may be provided. In this case, the two intermediate pressurizing portions D-300 may be disposed to face the two first pressurizing portions D-210 disposed in the center area of the first mold D-200. It is as described above that the intermediate pressurizing portions D-300 are disposed between the first mold D-200 and the second mold D-400.

In addition, in the case of Embodiment 3-2, two penetration portions D-420aa may be provided on the second plane portion D-420a of the second mold D-400. Accordingly, when the outer area of the metal sheet D-10A is press formed by the first mold D-200 and the second mold D-400, the two intermediate pressurizing portions D-300 may be housed in the penetration portions D-420aa, respectively.

In the "method for manufacturing a press formed part D-10' according to Embodiment 3-2" using the manufacturing apparatus D-20' as described above, S100, S200, S300, and S400 may be sequentially performed, like the method for manufacturing a press formed part D-10 of Embodiment 3-1. Herein, since the specific manufacturing method performed in each process is identical or similar to the case of Embodiment 3-1, description will focus on the difference.

First, in S100, a metal sheet D-10' may be supplied to the working position described above, as shown in FIG. 42. In this case, the metal sheet D-10A may be supplied to the manufacturing apparatus D-20', in a state of being heated by a separate heating apparatus (not shown). When supplied to the working position, two intermediate pressurizing portion D-300 may be placed under the center area of the metal sheet D-10'. Herein, the two intermediate pressurizing portion D-300 may be disposed at the same height. In this case, a height difference (hi) between the intermediate pressurizing portions D-300 and the second pressurizing portion D-410 may be the same as the case of Embodiment 3-1.

Next, in S200, as the first mold D-200 descends, the intermediate pressurizing portions D-300 are introduced into the two first pressurizing portions D-210 disposed in the center area of the first mold D-200, respectively, and may pressurize the center area of the metal sheet D-10', as shown in FIG. 43. Two deformation portions D-120 may be formed in the center area of the metal sheet D-10A, by the first press forming process.

Next, in S300, the first mold D-200 further descends, so that the two pressurizing portions D-410 may be introduced into the two first pressurizing portions D-210 disposed in the outer area of the first metal D-200, respectively, as shown in FIG. 44. Thus, the outer area of the metal sheet D-10' may be pressed in the up and down direction by the first pressurizing portion D-210 and the second pressurizing portion D-410. Two deformation portions D-120 may be further formed in the outer area of the metal sheet D-10A, by the second press forming process.

Next, in S400, the first mold D-200 may rise in the opposite direction +Z to the pressurizing direction -Z, as shown in FIG. 45. Accordingly, the press formed part D-10' in a state of completing press forming may be separated from the first mold C-200, the intermediate pressurizing portion D-300, and the second mold D-400. In this process, the two intermediate pressurizing portions D-300 may rise and return to its original position at the working position as described above.

Next, after the press formed part D-10' after manufacturing is discharged from the manufacturing apparatus D-20', a new metal sheet D-10' is supplied and the next press forming process may start.

Meanwhile, when the number of deformation portions D-120 formed in the press formed part D-10' increases, the number of intermediate pressurizing portions D-300 may also increase correspondingly.

For example, though not shown in the drawing, when 5 deformation portions D-120 are formed in the press formed part D-10', 5 first pressurizing portions D-210 should be provided in the first mold D-200. Accordingly, the three intermediate pressurizing portions D-300 may be disposed to face the three first pressurizing portions D-210 disposed in the center area of the first mold D-200. In this case, the three intermediate pressurizing portion D-300 may be disposed between the first mold D-200 and the second mold D-400.

Among the three intermediate pressurizing portions D-300, one intermediate pressurizing portion disposed in the center (hereinafter, referred to as first intermediate pressurizing portion) D-300 may be disposed at the highest position. The remaining two intermediate pressurizing portions (hereinafter, referred to as second intermediate pressurizing portions) D-300 may be disposed between the first intermediate pressurizing portion D-300 and the second mold D-400. Herein, the two second intermediate pressurizing portion D-300 may be disposed at the same height. A height difference between the first intermediate pressurizing portion D-300 and the second intermediate pressurizing portion D-300 may be identical or similar to the height difference (hi) between the intermediate pressurizing portion D-300 and the second pressurizing portion D-410 described above.

First, the first press forming may be performed in the state of being dispose, by the first mold D-200 and the first intermediate pressurizing portion D-300. After or immediately before the completion of the first press forming, the first mold D-200 further descends together with the first intermediate pressurizing portion D-300, thereby performing second press forming by the first mold D-200 and the two second intermediate pressurizing portion D-300. Forming of the center area of the metal sheet D-10A may be first performed by the two press forming. Thereafter, after or immediately before the completion of the second press forming, the first mold D-200 further descends, thereby performing third press forming by the outer area of the metal sheet D-10A by the first mold D-200 and the second mold D-400.

As another example, though not shown in the drawing, when 6 deformation portions D-120 are formed in the press formed part D-10', 6 first pressurizing portions D-210 should be provided in the first mold D-200. Accordingly, the four intermediate pressurizing portions D-300 may be disposed to face the four first pressurizing portions D-210 disposed in the center area of the first mold D-200. In this case, the four intermediate pressurizing portion D-300 may be disposed between the first mold D-200 and the second mold D-400.

Among the four intermediate pressurizing portions D-300, two intermediate pressurizing portions disposed in the center (hereinafter, referred to as first intermediate pressurizing portion) D-300 may be disposed at the highest position. The remaining two intermediate pressurizing portions (hereinafter, referred to as second intermediate pressurizing portions) D-300 may be disposed between the first intermediate pressurizing portion D-300 and the second mold D-400. Herein, the two first intermediate pressurizing portion D-300 may be disposed at the same height. Further, the two second intermediate pressurizing portion D-300 may be disposed at the same height. A height difference between the first intermediate pressurizing portion D-300 and the second intermediate pressurizing portion D-300 may be identical or similar to the height difference (hi) between the intermediate pressurizing portion D-300 and the second pressurizing portion D-410 described above.

First, the first press forming may be performed in the state of being dispose, by the first mold D-200 and the two first intermediate pressurizing portions D-300. After or immediately before completion of the first press forming, the first mold D-200 further descends together with the first intermediate pressurizing portions D-300, thereby performing second press forming by the first mold D-200 and the two second intermediate pressurizing portions D-300. Forming of the center area of the metal sheet D-10A may be first performed by the two press forming. Thereafter, after or immediately before the completion of the second press forming, the first mold D-200 further descends, thereby performing third press forming by the outer area of the metal sheet D-10A by the first mold D-200 and the second mold D-400.

In addition, when the number of deformation portions D-120 formed in the press formed part D-10' is increased to 7 or more, the number of the first pressurizing portions D-210 and the number of the intermediate pressurizing portions D-300 should be further increased, similarly to the above. Accordingly, the number of the penetration portions D-420aa in the second mold D-400 may be increased, of course. The press forming of the center area of the metal sheet D-10A is first performed by the method of adding a press forming process, in a state of configuring the manufacturing apparatus as such, and then the press forming of the outer area of the metal sheet D-10A may be performed.

In the press forming parts D-10 and D-10' according to example embodiments of the present disclosure as described above and the manufacturing method thereof (S10), the press forming may be performed on the metal sheets D-10 and D-10' by disposing the intermediate pressurizing portion D-300 having a height difference (hi) between the upper/loser molds D-200 and D-400 and using the three pressurizing portions D-210, D-300, and D-410. Herein, a strain being concentrated on a certain position of the metal sheets D-10 and D-10' during press working may be prevented by a stepwise forming process of first pressing the center area of the metal sheets D-10 and D-10', and then sequentially pressing the outer area. Thus, the press formed parts D-10 and D-10' are prevented from being damaged in the manufacturing process, and part quality may be improved.

Hereinabove, although the example embodiments of the present disclosure have been described with reference to the accompanying drawings, those skilled in the art will understand that various modifications and alterations may be made without departing from the spirit or essential feature of the present disclosure. Therefore it should be understood that the above-mentioned example embodiments are illustrative in all aspects and not restrictive.

### [Description of Reference Characters]

A-10: Upper Die
A-12: Cooling Channel
A-20: Lower Punch
A-22: Cooling Channel
A-30: Lower Holder
A-32: Heating Heater
A-34: Cooling Channel
A-100: Mold
A-200: Steel Material
A-300: 22MnB5 Material
B-1: Side frame B-10: Frame
B-20: Bracket B-21, 22: Flange
B-23: Main Body B-24: Curved Surface
B-100: Punch
B-110, B-120, B-130, B-140, B-150: First to Fifth Punch Forming Portions
B-111, B-121, B-131, B-141, B-151: First to Fifth extended surface forming portions
B-112, B-122, B-132, B-142, B-152: First to Fifth Curved Surface Forming portions
B-113, B-123, B-133, B-143: First to Fourth Main Body forming portions
B-200: Pad
B-300: Die
B-310, B-320, B-330, B-340, B-350: First to Fifth die forming portions
B-311, B-321, B-331, B-341, B-351: First to Fifth Die Curved Surface Forming Portions
B-312, B-322, B-332, B-342, B-352: First to Fifth Die Plane Forming Portions
B-360: Vertical Plane
B-400: Material B-410: Notch
C-1: Battery pack module C-10: Hot Press Formed Part
C-20: Battery case C-30: Base
C-40: Reinforcing Member C-110: First Wall
C-120: Second Wall C-130: Third Wall
C-140: Fourth Wall C-150: Fifth Wall
C-160: Curvature Portion C-170: First Connection Portion
C-180: Second Connection Portion C-190: Third Connection Portion
b: Battery Pack r: Radius of Curvature
t: Sheet Material Thickness θw: Wall Portion Angle
hw: Wall Portion Height
D-10, D-10': Press Formed part
D-10A: Metal Sheet
D-110: Flat Plate Portion
D-120: Deformation Portion
D-20, D-20': Press Formed Apparatus
D-200: First Mold
D-210: First Protrusion
D-220: First Plane Portion
D-300: Intermediate Pressurizing Portion
D-400: Second Mold
D-410: Second Protrusion
D-420: Second Plane Portion

### Mode for Invention

Hereinafter, the present disclosure will be described in detail by way of the examples. However, it should be noted that the following examples are only for describing the present disclosure by illustration, and not intended to limit the scope of right of the present disclosure. The reason is that the right scope of the present disclosure is determined by the matters described in the claims and reasonably inferred therefrom.

### (Example 1)

Steel slabs which had an alloy composition shown in the following Table 2 and had a thickness of 100 mm were manufactured by vacuum melting. Each steel slab was heated to 1250°C, finish hot rolled at 900°C, cooled at a cooling rate of 30°C/s, and then coiled at 640°C, thereby obtaining a hot rolled steel sheet having a final thickness of 2.5 mm. Thereafter, each hot rolled steel sheet was pickled and cold rolled under the conditions shown in Table 2 to manufacture a cold rolled steel sheet. At this time, a total rolling reduction rate during cold rolling was set to 45%. Thereafter, each cold rolled steel sheet was annealed at an annealing temperature of 780°C under the atmosphere of 5% hydrogen - 95% nitrogen and then cooled to manufacture an annealing cold rolled steel sheet.

Each annealing cold rolled steel sheet manufactured as described above was manufactured into a blank, and then hot forming and cooled using a mold for hot forming to obtain a hot formed member. At this time, the heating temperature of the blank was 900°C, the maintenance time at the temperature was set to 5 minutes, and the cooling rate was 40°C/s.

As such, in performing the hot forming, a transfer time from a heating furnace to hot forming using the mold was identically applied as 10 seconds.

The physical properties of each of the annealed cold rolled steel sheet (steel material for hot forming) described above and the hot formed member were measured.

Specifically, for the annealed cold rolled steel sheet, the strength of a rotated-cube texture on an orientation distribution function (ODF) map and the colony area fraction of surfaces perpendicular to the <111> direction in the thickness direction were measured by applying an electron backscattered diffraction (EBSD) technique. For data analysis, the ODF map on ferrite was configured using the EDAX OIM Analysis^{™} v7.3 program, and the derived values are shown in the following Table 3. At this time, a deviation of angle of orientation for measuring the colony area fraction was set to ±5°, and then the area fraction was calculated.

In addition, in order to evaluate the bending anisotropy of the hot formed member, the bendability evaluation according to the VDA238-100 standard was performed. Specifically, when the deviation in bending angle which was derived from [Equation 1] after performing a 3-point bending test was more than 15.0, the anisotropy was evaluated as being poor. [Equation 1] {|Bending angle in rolling perpendicular direction - bending angle in rolling direction|/bending angle in rolling direction}×100.

Further, the mechanical properties (tensile strength (TS), yield strength (YS), and elongation (EI)) were measured using a universal tensile tester in accordance with the ISO6892 standard with a specimen No. JIS-5.

**[Table 2]**

| Steel type | Alloy composition (wt%) | | | | | | | |
|---|---|---|---|---|---|---|---|---|
| | C | Si | Mn | P | S | Al | Cr | N |
| A | 0.435 | 1.79 | 1.54 | 0.007 | 0.004 | 0.06 | 2.120 | 0.004 |
| B | 0.311 | 1.20 | 1.87 | 0.003 | 0.003 | 0.06 | 3.990 | 0.008 |
| C | 0.207 | 1.05 | 1.48 | 0.009 | 0.010 | 0.08 | 1.157 | 0.003 |
| D | 0.084 | 1.09 | 1.00 | 0.005 | 0.007 | 0.01 | 3.610 | 0.008 |
| E | 0.375 | 2.71 | 1.25 | 0.008 | 0.005 | 0.04 | 4.291 | 0.003 |

**[Table 3]**

| Steel type | Rolling reduction rate (%) of first cold rolling mill | Rolling reduction rate (%) of last cold rolling mill | Classification |
|---|---|---|---|
| A | 19.39 | 8.61 | Inventive Example A-1 |
| A | 2.77 | 0.07 | Comparative Example A-1 |
| A | 0.39 | 3.28 | Comparative Example A-2 |
| A | 8.10 | 0.03 | Comparative Example A-3 |
| B | 14.51 | 5.88 | Inventive Example A-2 |
| B | 4.88 | 6.29 | Comparative Example A-4 |
| B | 24.46 | 0.07 | Comparative Example A-5 |
| C | 30.70 | 3.50 | Inventive Example A-3 |
| C | 4.71 | 0.06 | Comparative Example A-6 |
| C | 2.76 | 1.20 | Comparative Example A-7 |
| C | 32.57 | 0.02 | Comparative Example A-8 |
| D | 25.80 | 8.81 | Inventive Example A-4 |
| D | 1.43 | 0.09 | Comparative Example A-9 |
| D | 3.16 | 3.84 | Comparative Example A-10 |
| D | 30.41 | 0.08 | Comparative Example A-11 |
| E | 15.98 | 3.70 | Inventive Example A-5 |
| E | 1.39 | 0.01 | Comparative Example A-12 |
| E | 2.80 | 5.25 | Comparative Example A-13 |
| E | 22.92 | 0.09 | Comparative Example A-14 |

**[Table 4]**

| Classification | Steel material for hot forming (annealed cold rolled steel sheet) | | Hot formed member | | | | | |
|---|---|---|---|---|---|---|---|---|
| | Rotated-cube strength | <111> perpendic ular plane colony area (%) | YS (MPa) | TS (MPa) | El (%) | Bending angle (°) in rolling perpendicular direction | Bending angle (°) in rolling direction | Deviation in bending angle (%) |
| Inventive Example A-1 | 2.11 | 17.20 | 1341 | 1970 | 5.9 | 43.0 | 43.9 | 2.1 |
| Comparative Example A-1 | 3.60 | 5.90 | 1013 | 1818 | 4.0 | 26.2 | 41.2 | 36.4 |
| Comparative Example A-2 | 2.96 | 2.69 | 1299 | 1858 | 6.2 | 35.9 | 42.6 | 15.7 |
| Comparative Example A-3 | 1.73 | 4.74 | 1349 | 1996 | 6.3 | 32.9 | 40.6 | 19.0 |
| Inventive Example A-2 | 1.85 | 9.56 | 1305 | 1860 | 6.4 | 44.0 | 48.5 | 9.3 |
| Comparative Example A-4 | 9.88 | 2.96 | 1081 | 1742 | 6.7 | 31.0 | 37.7 | 17.8 |
| Comparative Example A-5 | 3.75 | 9.27 | 1110 | 1786 | 6.7 | 31.3 | 37.9 | 17.4 |
| Inventive Example A-3 | 2.14 | 7.98 | 1053 | 1489 | 7.3 | 56.4 | 56.9 | 0.9 |
| Comparative Example A-6 | 1.12 | 5.93 | 1074 | 1525 | 7.2 | 42.8 | 58.0 | 26.2 |
| Comparative Example A-7 | 8.14 | 3.29 | 1061 | 1516 | 6.9 | 46.6 | 56.7 | 17.8 |
| Comparative Example A-8 | 3.31 | 7.89 | 1057 | 1507 | 7.6 | 46.8 | 55.8 | 16.1 |
| Inventive Example A-4 | 1.52 | 9.24 | 855 | 1100 | 6.9 | 100.1 | 100.8 | 0.7 |
| Comparative Example A-9 | 4.70 | 2.49 | 848 | 1091 | 7.0 | 84.7 | 102.5 | 17.4 |
| Comparative Example A-10 | 1.05 | 4.08 | 886 | 1113 | 5.9 | 76.7 | 104.0 | 26.3 |
| Comparative Example A-11 | 4.30 | 6.33 | 813 | 1049 | 7.1 | 86.9 | 105.0 | 17.2 |
| Inventive Example A-5 | 2.34 | 8.05 | 1341 | 1973 | 7.1 | 57.9 | 57.6 | 0.5 |
| Comparative Example A-12 | 8.03 | 4.17 | 1390 | 2037 | 7.3 | 48.1 | 57.5 | 16.3 |
| Comparative Example A-13 | 3.11 | 6.12 | 1396 | 2079 | 7.0 | 43.9 | 52.1 | 15.7 |
| Comparative Example A-14 | 2.33 | 4.49 | 1389 | 2030 | 7.4 | 45.5 | 53.8 | 15.4 |

As shown in Tables 2 to 4, in Inventive Examples A-1 to A-5 satisfying the alloy composition and the manufacturing conditions (in particular, cold rolling conditions), the strength of the rotated-cube on the ODF map of ferrite was 2.50 or less, and the colony fraction of the surfaces perpendicular to the <111> direction in the thickness direction was more than 6.00 in the steel material for hot forming (annealed cold rolled steel sheet). Thus, the bending anisotropy of the hot formed member obtained by hot forming the steel material for hot forming was able to be secured excellently.

However, Comparative Examples A-1 to A-14 in which all alloy compositions satisfied the present disclosure, but the manufacturing conditions (cold rolling conditions) were out of the scope of the present disclosure, were not able to secure the characteristics of the steel material for hot forming. Thus, the deviation in bending angle in the hot formed member was more than 15.0, and thus, the bending anisotropy was confirmed to be poor.

FIG. 1 shows the results of the ODF map of Inventive Example A-1 and Comparative Example A-1, in which the color on the drawing goes from blue to red, the colony area was increased, and the value is as described.

As shown in FIG. 1, it was confirmed that the colony area fraction of the surfaces perpendicular to the <111> direction in Inventive Example A-1 was higher than that in Comparative Example A-1.

### (Example 2)

Steel slabs which had an alloy composition shown in the following Table 5 and had a thickness of 100 mm were manufactured by vacuum melting. Each steel slab was heated to 1250°C, finish hot rolled at 900°C, cooled at a cooling rate of 30°C/s, and then coiled at 640°C, thereby obtaining a hot rolled steel sheet having a final thickness of 2.5 mm. Thereafter, each hot rolled steel sheet was pickled and cold rolled at a rolling reduction rate of 45% to manufacture a cold rolled steel sheet. Thereafter, each cold rolled steel sheet was annealed at an annealing temperature of 780°C under the atmosphere of 5% hydrogen - 95% nitrogen and then cooled to manufacture an annealing cold rolled steel sheet.

Each annealed cold rolled steel sheet manufactured as described above was manufactured into a blank, the blank was transferred into a heating furnace, and then hot formed and cooled according to the conditions shown in Table 6, using a mold for hot forming to obtain a hot formed member.

The microstructure, surface quality, physical properties, and the like of each hot formed member were evaluated and shown in the following Table 7.

Specifically, in order to measure the microstructure of the hot formed member, a specimen cross section at a t/4 point in the thickness direction was polished and etched, and then observed using a scanning electron microscope (SEM), and at this time, magnification was performed 10,000 times for cementite size analysis, and long and short diameters were measured. In addition, the composition of the cementite was measured at 10,000x magnification, using energy dispersive X-ray spectroscopy (EDS).

In addition, in order to inspect surface quality of the hot formed member, the surface glossiness (angle between an incident angle and a member surface normal vector of 60°) of each member surface was measured in accordance with the ISO2813 standard, and in order to evaluate the tensile physical properties, a tensile test at room temperature was performed with a specimen No. JIS-5 in accordance with ISO6892.

Further, for bendability evaluation, bendability evaluation according to the VDA238-100 standard was performed to determine a maximum bending angle. At this time, an angle at which the maximum bending strength specified in the specification was secured was measured, and then converted into the bending angle to derive a maximum bending angle, and the value is shown.

**[Table 5]**

| Steel type | Alloy composition (wt%) | | | | | | | | | |
|---|---|---|---|---|---|---|---|---|---|---|
| | C | Si | Mn | P | S | Al | Cr | Ti | B | N |
| F | 0.345 | 0.20 | 1.25 | 0.010 | 0.0010 | 0.035 | 0.40 | 0.030 | 0.0025 | 0.003 |
| G | 0.291 | 0.00 | 0.01 | 0.010 | 0.0020 | 0.053 | 2.00 | 0.016 | 0.0018 | 0.001 |
| H | 0.290 | 0.50 | 0.01 | 0.010 | 0.0030 | 0.050 | 1. 90 | 0.015 | 0.0020 | 0.002 |
| I | 0.293 | 1.49 | 0.59 | 0.010 | 0.0008 | 0.046 | 0.69 | 0.015 | 0.0029 | 0.004 |
| J | 0.070 | 0.96 | 0.02 | 0.010 | 0.0030 | 0.051 | 1. 93 | 0.015 | 0.0020 | 0.001 |
| K | 0.250 | 1.53 | 0.39 | 0.010 | 0.0008 | 0.035 | 1.00 | 0.014 | 0.0025 | 0.004 |
| L | 0.314 | 1.50 | 0.08 | 0.010 | 0.0006 | 0.057 | 1.50 | 0.015 | 0.0026 | 0.003 |
| M | 0.254 | 1.49 | 0.79 | 0.010 | 0.0020 | 0.0405 | 4.32 | 0.032 | 0.0028 | 0.005 |

**[Table 6]**

| Steel type | Ae3 (°C) | Heating furnace condition | | | | Relation 1 | Relation 2 | Steel No. |
|---|---|---|---|---|---|---|---|---|
| | | Oxygen concentration (%) | Dew point temperature (°C) | T_{furnace} (°C) | tₜₒₜₐₗ (sec) | | | |
| F | 780 | 5 | 5 | 900 | 500 | 0.15 | 142.6 | 1 |
| G | 810 | 5 | 5 | 900 | 400 | 0.23 | 163.6 | 2 |
| H | 821 | 5 | 5 | 900 | 400 | 0.45 | 173.3 | 3 |
| I | 851 | 5 | 5 | 900 | 400 | 0.40 | 210.8 | 4 |
| J | 918 | 5 | 5 | 950 | 300 | 0.90 | 248.5 | 5 |
| J | 918 | 20 | 5 | 950 | 400 | -2.19 | 248.5 | 6 |
| J | 918 | 5 | 10 | 950 | 400 | 0.60 | 248.5 | 7 |
| K | 880 | 1 | 5 | 900 | 400 | 1.32 | 300.4 | 8 |
| K | 880 | 1 | 5 | 900 | 150 | 1. 60 | 300.4 | 9 |
| K | 880 | 1 | 5 | 900 | 1000 | 0.48 | 300.4 | 10 |
| K | 880 | 5 | 5 | 900 | 400 | 0.54 | 300.4 | 11 |
| L | 854 | 1 | 5 | 900 | 400 | 1.49 | 216.1 | 12 |
| L | 854 | 5 | 5 | 900 | 400 | 0.70 | 216.1 | 13 |
| M | 827 | 5 | 5 | 900 | 400 | 6.87 | 179.3 | 14 |
| M | 827 | 5 | 5 | 950 | 100 | 7.17 | 140.8 | 15 |
| - In Table 6, the Aₑ₃ temperature is a value calculated using a Thermo_calc. Software, and at this time, TCFE6 was applied as the database. | | | | | | | | |
| - The value of Relation 1 is a value rounded off from the third decimal place, and the value of Relation 2 is a value rounded off from the second decimal place. | | | | | | | | |

**[Table 7]**

| Steel No. | Structural characteristics | | Tensile properties | | | | Glossines s (GU) | Maximum bending angle (°) | Classification |
|---|---|---|---|---|---|---|---|---|---|
| | Ferrite fraction (% by area) | Number of cementites (/µm) | YS (MPa) | TS (MPa) | YR | El (%) | | | |
| 1 | 0.0 | 8.47 | 1324 | 1983 | 0.67 | 6.1 | 3.8 | 45 | Inventive Example B-1 |
| 2 | 0.0 | 3.45 | 1152 | 1662 | 0.69 | 7.6 | 5.6 | 56 | Inventive Example B-2 |
| 3 | 0.0 | 4.06 | 1134 | 1713 | 0.66 | 7.8 | 11.3 | 53 | Inventive Example B-3 |
| 4 | 0.0 | 3.59 | 1272 | 1902 | 0.67 | 7.1 | 10.1 | 48 | Inventive Example B-4 |
| 5 | 0.0 | 4.78 | 791 | 1165 | 0.68 | 7.7 | 27.9 | 83 | Inventive Example B-5 |
| 6 | 0.0 | 3.57 | 787 | 1141 | 0.69 | 7.0 | -54.9 | 82 | Inventive Example B-6 |
| 7 | 0.0 | 4.57 | 759 | 1143 | 0.66 | 7.1 | 15.1 | 84 | Inventive Example B-7 |
| 8 | 0.0 | 3.89 | 1182 | 1754 | 0.67 | 7.2 | 33.1 | 53 | Inventive Example B-8 |
| 9 | 8.1 | 12.30 | 858 | 1252 | 0.69 | 11.2 | 41.8 | 31 | Comparative Examples B-1 |
| 10 | 0.0 | 0.87 | 1146 | 1690 | 0.68 | 7.8 | 12.1 | 55 | Inventive Example B-9 |
| 11 | 0.0 | 4.54 | 1186 | 1756 | 0.68 | 6.3 | 13.4 | 52 | Inventive Example B-10 |
| 12 | 0.0 | 3.98 | 1291 | 1899 | 0.68 | 7.4 | 37.3 | 47 | Inventive Example B-11 |
| 13 | 0.0 | 3.25 | 1307 | 1905 | 0.69 | 7.9 | 17.6 | 46 | Inventive Example B-12 |
| 14 | 0.0 | 3.16 | 1232 | 1797 | 0.69 | 7.9 | 171.8 | 52 | Inventive Example B-13 |
| 15 | 11.2 | 18.30 | 765 | 1121 | 0.68 | 11.2 | 179.3 | 34 | Comparative Examples B-2 |
| - Among the structural characteristics, the remaining structure other than a ferrite fraction was a martensite phase in all examples. That is, when the ferrite fraction was 0%, it means that the microstructure was a martensite single phase structure. | | | | | | | | | |
| - The number of cementites refers to the number of cementites in which the Cr content was 1.20% or more and the length of the short diameter was 100 nm or more, at a t/4 point in the thickness direction. | | | | | | | | | |

As shown in Tables 5 to 7, Inventive Examples B-1 to B-13 having the number of specific cementites of 10.00 µm² or less according to an example embodiment of the present disclosure had the results of bending characteristics of 40° or more and was confirmed to have excellent bendability.

Among them, the examples in which some were out of the scopes of the alloy composition according to an example embodiment of the present disclosure and/or the manufacturing conditions according to an example embodiment of the present disclosure showed a glossiness of less than 25.0 GU.

However, the examples in which the alloy composition and the manufacturing conditions according to an example embodiment of the present disclosure were all satisfied (Inventive Examples B-5, B-8, B-11, and B-13) showed excellent results of surface quality as well as bendability.

Meanwhile, Comparative Examples B-1 and B-2 having the number of specific cementites of more than 10.00 µm² according to an example embodiment of the present disclosure showed poor results of bendability. Since Comparative Examples B-1 and B-2 were stayed in the furnace for a shorter time than the value derived by Relation 2, that is, a heat treatment time was not sufficient, specific cementite was excessively formed, and also ferrite in the microstructure was transformed to deteriorate bendability.

FIG. 2 is photographs in which the surfaces of Inventive Example B-5 and Inventive Example B-1 were observed. As shown in FIG. 2, it was confirmed that the surface quality of Inventive Example B-5 was better than that of Inventive Example B-1, even with the naked eye.

### (Example 3)

### Inventive Example C

A steel material having a martensite transformation critical cooling rate of 18°C/s in the temperature section of 800 to 400°C was heated to 930°C, maintained for 60 seconds, and then air cooled to 730°C at a cooling rate of 15°C/s. Thereafter, the steel material was provided in hot press forming equipment as shown in FIG. 8, a blank holding force (F) and heat were applied through a lower holder to support the steel material between the lower holder and the upper die and also heat it. At this time, the blank holding pressure (P) was 5 MPa, and the contact area (A) of the lower holder and the steel material was 30000 mm². That is, the blank holding force (F) was 150 kN. The temperature of the lower holder was 600°C. The forming temperature (T_{blank}) of the steel material was 730°C, the thickness (w) of the steel material was 1.5 mm, the density (ρ) of the steel material was 7.7×10⁻⁹ ton/mm³, and the specific heat (C) of the steel material was 6.7×10⁸ mJ/ton·K. The heat transfer pressurization coefficient (a) of the steel material was 2.3, and the heat transfer pressurization index (b) was 0.18. Thereafter, the steel material was formed, and cooled at a cooling rate of 20°C/s. Meanwhile, the temperature of all molds other than the lower holder was set to 80°C. The results of measuring the flange portion wrinkle wave height of the hot press formed part manufactured therefrom was 0.5 mm. At this time, the wave height was calculated as a difference between a maximum height and a minimum height for the flange portion wrinkles.

### Comparative Example C

FIG. 9 is a schematic diagram showing hot press forming equipment applied to the 22MnB5 material. The 22MnB5 material A-300 was heated to 930°C, maintained for 60 seconds, and air cooled to 730°C at a cooling rate of 15°C/s. Thereafter, the 22MnB5 material A-300 was provided in the hot press forming equipment as shown in FIG. 7, and the steel material was formed and cooled at a cooling rate of 50°C/s. At this time, a gap between the upper die and the lower holder was set to 3 mm, and the temperature of the entire mold was set to 80°C. The results of measuring the flange portion wrinkle wave height of the hot press formed part manufactured therefrom was 3.0mm. At this time, the wave height was calculated as a difference between a maximum height and a minimum height for the flange portion wrinkles.

Hereinabove, though the present disclosure has been described with reference to the examples, the present disclosure is not limited to the examples and may be modified by those skilled in the art without changing technical idea of the present disclosure claimed below.

## Claims

1. A steel material for hot forming, wherein a strength of rotated-cube texture on an orientation distribution function (ODF) map is 2.50 or less, and a colony of surfaces perpendicular to a <111> direction in a thickness direction is more than 6.00% of an entire texture area.

2. The steel material for hot forming of claim 1, wherein the steel material includes, by weight: 0.040 to 0.450% of carbon (C), 0.80 to 3.00% of silicon (Si), 4.00% or less (excluding 0%) of manganese (Mn), 0.050% or less of phosphorus (P), 0.0200% or less of sulfur (S), 0.010 to 0.100% of aluminum (Al), 1.000 to 5.000% of chromium (Cr), 0.020% or less (excluding 0%) of nitrogen (N), a reminder of Fe, and unavoidable impurities.

3. The steel material for hot forming of claim 1, wherein the steel material further includes one or more elements selected from the following a) to f):
a) 0.005 to 0.400 wt% of one or more selected from titanium (Ti), niobium (Nb), zirconium (Zr), and vanadium (V),
b) 0.0001 to 0.0100 wt% of boron (B),
c) 0.001 to 1.000 wt% of one or more of molybdenum (Mo) and tungsten (W),
d) 0.003 to 2.000 wt% of one or more of copper (Cu) and nickel (Ni),
e) 0.001 to 1.000 wt% of one or more of antimony (Sb) and tin (Sn), and
f) 0.0001 to 0.0200 wt% of rare earth elements (REM).

4. The steel material for hot forming of claim 1,
wherein a microstructure of the steel material includes ferrite or a composite structure of ferrite and cementite as a main phase, and additionally, one or more of pearlite, bainite, and martensite, and
the main phase is included at an area fraction of 30% or more.

5. The steel material for hot forming of claim 1, wherein the steel material has a tensile strength of 550 MPa or more.

6. A method for manufacturing a steel material for hot rolling, the method comprising:
preparing a steel slab;
heating the steel slab in a temperature range of 1000 to 1300°C;
performing finish hot rolling of the heated steel slab in a temperature range of Ar3 to 1000°C to obtain a hot rolled steel sheet;
after the finish hot rolling, performing cooling at a cooling rate of 20 to 100°C/s;
after the cooling, performing coiling in a temperature range of higher than Ms and 750°C or lower;
after the coiling, performing cold rolling to obtain a cold rolled steel sheet; and
annealing the cold rolled steel sheet in a temperature range of 700 to 900°C,
wherein the cold rolling is performed at a rolling reduction rate of 5% or more and less than 35% in a first cold rolling mill and at a rolling reduction rate of 0.1% or more and less than 10.0% in a last cold rolling mill.

7. The method for manufacturing a steel material for hot rolling of claim 6, wherein the steel slab includes, by weight: 0.040 to 0.450% of carbon (C), 0.80 to 3.00% of silicon (Si), 4.00% or less (excluding 0%) of manganese (Mn), 0.050% or less of phosphorus (P), 0.0200% or less of sulfur (S), 0.010 to 0.100% of aluminum (Al), 1.000 to 5.000% of chromium (Cr), 0.020% or less (excluding 0%) of nitrogen (N), a reminder of Fe, and unavoidable impurities.

8. The method for manufacturing a steel material for hot rolling of claim 6, wherein the steel slab further includes one or more elements selected from the following a) to f):
a) 0.005 to 0.400 wt% of one or more selected from titanium (Ti), niobium (Nb), zirconium (Zr), and vanadium (V),
b) 0.0001 to 0.0100 wt% of boron (B),
c) 0.001 to 1.000 wt% of one or more of molybdenum (Mo) and tungsten (W),
d) 0.003 to 2.000 wt% of one or more of copper (Cu) and nickel (Ni),
e) 0.001 to 1.000 wt% of one or more of antimony (Sb) and tin (Sn), and
f) 0.0001 to 0.0200 wt% of rare earth elements (REM).

9. A hot formed member wherein [Equation 1] satisfies 15.0 or less: {|Bending angle in rolling perpendicular direction - bending angle in rolling direction|/bending angle in rolling direction}×100.

10. The hot formed member of claim 9, wherein the member includes, by weight: 0.040 to 0.450% of carbon (C), 0.80 to 3.00% of silicon (Si), 4.00% or less (excluding 0%) of manganese (Mn), 0.050% or less of phosphorus (P), 0.0200% or less of sulfur (S), 0.010 to 0.100% of aluminum (Al), 1.000 to 5.000% of chromium (Cr), 0.020% or less (excluding 0%) of nitrogen (N), a reminder of Fe, and unavoidable impurities.

11. The hot formed member of claim 9, wherein the member is a martensite single phase or a composite structure of bainite at an area fraction of 40% or less and a remainder of martensite.

12. The hot formed member of claim 9, wherein the member further includes one or more elements selected from the following a) to f):
a) 0.005 to 0.400 wt% of one or more selected from titanium (Ti), niobium (Nb), zirconium (Zr), and vanadium (V),
b) 0.0001 to 0.0100 wt% of boron (B),
c) 0.001 to 1.000 wt% of one or more of molybdenum (Mo) and tungsten (W),
d) 0.003 to 2.000 wt% of one or more of copper (Cu) and nickel (Ni),
e) 0.001 to 1.000 wt% of one or more of antimony (Sb) and tin (Sn), and
f) 0.0001 to 0.0200 wt% of rare earth elements (REM).
